



US008129310B2

(12) **United States Patent**  
**Yokozawa**

(10) **Patent No.:** **US 8,129,310 B2**  
(45) **Date of Patent:** **Mar. 6, 2012**

(54) **HEAT-SENSITIVE TRANSFER SHEET**

(75) Inventor: **Akito Yokozawa**, Minami-ashigara (JP)

(73) Assignee: **Fujifilm Corporation**, Tokyo (JP)

(\*) Notice: Subject to any disclaimer, the term of this patent is extended or adjusted under 35 U.S.C. 154(b) by 758 days.

(21) Appl. No.: **12/239,553**

(22) Filed: **Sep. 26, 2008**

(65) **Prior Publication Data**

US 2009/0087598 A1 Apr. 2, 2009

(30) **Foreign Application Priority Data**

Sep. 28, 2007 (JP) ..... 2007-255793

(51) **Int. Cl.**

*B41M 5/035* (2006.01)  
*B41M 5/382* (2006.01)

(52) **U.S. Cl.** ..... **503/227; 8/471**

(58) **Field of Classification Search** ..... None  
See application file for complete search history.

(56) **References Cited**

U.S. PATENT DOCUMENTS

|                 |         |                      |
|-----------------|---------|----------------------|
| 4,961,997 A     | 10/1990 | Asano et al.         |
| 5,073,533 A *   | 12/1991 | Aono .....           |
| 7,678,739 B2 *  | 3/2010  | Hashiba et al. ..... |
| 7,833,938 B2 *  | 11/2010 | Yunoki et al. .....  |
| 2005/0054527 A1 | 3/2005  | Iwasaki et al.       |

FOREIGN PATENT DOCUMENTS

|    |               |         |
|----|---------------|---------|
| JP | 62-259889 A   | 11/1987 |
| JP | 08-002123 *   | 1/1996  |
| JP | 8-90945 A     | 4/1996  |
| JP | 11-20325 A    | 1/1999  |
| JP | 2002-278149 A | 9/2002  |
| JP | 3410157 B2    | 3/2003  |
| JP | 2006-306016 A | 11/2006 |
| JP | 201163488 A   | 3/2011  |

OTHER PUBLICATIONS

“Hakuenga DD”; Shiraishi Kogyo Kaisha, Ltd.; Aug. 2006; XP-002555451; URL: <http://www.shiraishi.co.jp/kogyo/english/applications/img/dd.pdf>.

\* cited by examiner

*Primary Examiner* — Bruce H Hess

(74) *Attorney, Agent, or Firm* — Sughrue Mion, PLLC

(57) **ABSTRACT**

A heat-sensitive transfer sheet containing a base film, a dye layer formed over one surface of the base film and containing a heat-transferable dye and a resin, and a heat-resistant lubricating layer formed over the other surface of the base film and containing inorganic particles and a resin, wherein the inorganic particles contained in the heat-resistant lubricating layer has a Mohs' hardness of 3 to 7 and a mean particle size of 0.3 to 5  $\mu\text{m}$ , and the ratio of the maximum width of each of the inorganic particles to the sphere equivalent diameter thereof is from 1.5 to 50.

**11 Claims, No Drawings**

## 1

## HEAT-SENSITIVE TRANSFER SHEET

## FIELD OF THE INVENTION

The present invention relates to a heat-sensitive transfer sheet, more specifically a heat-sensitive transfer sheet which is restrained from being deformed in high-speed printing and simultaneously causes the amount of materials adhering to a thermal printer head to be decreased so as to overcome defects of images or cutting of the sheet.

## BACKGROUND OF THE INVENTION

Various heat transfer recording methods have been known so far. Among these methods, dye diffusion transfer recording systems attract attention as a process that can produce a color hard copy having an image quality closest to that of silver halide photography. Moreover, this system has advantages over silver halide photography: it is a dry system, it enables direct visualization from digital data, it makes reproduction simple, and the like.

In this dye diffusion transfer recording system, a heat-sensitive transfer sheet (hereinafter also referred to as an ink sheet) containing dyes is superposed on a heat-sensitive transfer image-receiving sheet (hereinafter also referred to as an image-receiving sheet), and then the ink sheet is heated by a thermal head whose exothermic action is controlled by electric signals, in order to transfer the dyes contained in the ink sheet to the image-receiving sheet, thereby recording an image information. Three colors: cyan, magenta, and yellow, are used for recording a color image by overlapping one color to other, thereby enabling transferring and recording a color image having continuous gradation for color densities.

Recently, various printers allowing higher-speed printing have been developed and commercialized increasingly in the field of the dye-diffusion transfer recording systems. The high speed print enables to shorten a waiting time when a user obtains a print in a shop. For the foregoing reason, there is a demand for further speeding up of printing.

In order to prevent thermal sticking between a thermal printer head of a printer and a heat-sensitive transfer sheet and to give the thermal printer head and the heat-sensitive transfer sheet a slipping property therebetween, a heat-resistant lubricating layer is formed on the heat-sensitive transfer sheet surface contacting the thermal printer head. The thermal sticking occurs in a case where there is a break of the ink ribbon or the slipping property of the ink ribbon is insufficient when an image is printed, whereby image defects may be generated because the heat-sensitive transfer sheet is stretched or creased, or deformed into some other form at the printing time. According to high-speed printing, a thermal printer head comes to contact the heat-resistant lubricating layer at a higher temperature and a higher speed. Thus, the heat-resistant lubricating layer is desired to have even better performances.

For example, Japanese Patent No. 3,410,157 discloses a technique of incorporating a phosphate ester (also called phosphate or phosphoric ester) surfactant, which is excellent in lubricity, into a lubricating layer, and incorporating magnesium hydroxide and particles having a Mohs' hardness less than 3 as neutralizing agents into the layer in order to restrain corrosion or abrasion of a thermal printer head by decomposition of the phosphate ester. Moreover, JP-A-8-90945 ("JP-A" means unexamined published Japanese patent publication) discloses a technique of incorporating, into an inorganic filler contained in a heat-resistant lubricating layer, a hard

## 2

impurity component in a certain amount range, thereby restraining creases or an abrasion of a thermal printer head.

The above-mentioned techniques have been used to investigate an improvement in performances of a heat-resistant lubricating layer in high-speed printing, so as to find out that the following cases may be caused: a case where the lubricity between a thermal printer head and the heat-resistant lubricating layer of a heat-sensitive transfer sheet is insufficient so that the heat-sensitive transfer sheet is not restrained from being deformed when an image is formed; and a case where refuses or residues adhering to a thermal printer head injure or damage the heat-sensitive transfer sheet when an image is formed, whereby the sheet is cut. The deformation of the heat-sensitive transfer sheet causes creases or other image defects when an image is printed; thus, the deformation is required to be overcome. Moreover, the cutting of the heat-sensitive transfer sheet causes an abnormal stop of the printer; thus, the cutting is also required to be overcome.

## SUMMARY OF THE INVENTION

The present invention resides in a heat-sensitive transfer sheet comprising a base film, a dye layer formed over one surface of the base film and containing a heat-transferable dye and a resin, and a heat-resistant lubricating layer formed over the other surface of the base film and containing inorganic particles and a resin, wherein the inorganic particles contained in the heat-resistant lubricating layer has a Mohs' hardness of 3 to 7 and a mean particle size of 0.3 to 5  $\mu\text{m}$ , and the ratio of the maximum width of each of the inorganic particles to the sphere equivalent diameter thereof is from 1.5 to 50.

Other and further features and advantages of the invention will appear more fully from the following description.

## DETAILED DESCRIPTION OF THE INVENTION

According to the present invention, there is provided the following means:

(1) A heat-sensitive transfer sheet comprising a base film, a dye layer formed over one surface of the base film and containing a heat-transferable dye and a resin, and a heat-resistant lubricating layer formed over the other surface of the base film and containing inorganic particles and a resin, wherein the inorganic particles contained in the heat-resistant lubricating layer has a Mohs' hardness of 3 to 7 and a mean particle size of 0.3 to 5  $\mu\text{m}$ , and the ratio of the maximum width of each of the inorganic particles to the sphere equivalent diameter thereof is from 1.5 to 50.

(2) The heat-sensitive transfer sheet according to item (1), wherein the Mohs' hardness ranges from 3 to 6.

(3) The heat-sensitive transfer sheet according to item (1) or (2), wherein the shape of the inorganic particles is tabular.

(4) The heat-sensitive transfer sheet according to item (1) or (2), wherein the inorganic particles contain particles in at least two forms which include tabular particles and needle particles.

(5) The heat-sensitive transfer sheet according to any one of items (1) to (4), wherein the ratio of the mass of the inorganic particles to the total coating mass of the heat-resistant lubricating layer is from 0.01% to 2 mass %.

(6) The heat-sensitive transfer sheet according to any one of items (1) to (5), wherein the inorganic particles are made of magnesium oxide.

(7) The heat-sensitive transfer sheet according to any one of items (1) to (6), wherein the above-described heat-sensitive

transfer sheet contains at least one dye represented by any one of following formulae (Y1) to (Y9) set forth below:



Formula (Y1) 5

wherein the ring A represents a substituted or unsubstituted benzene ring; R<sup>1</sup> and R<sup>2</sup> each independently represent a hydrogen atom, a substituted or unsubstituted alkyl group, a substituted or unsubstituted alkenyl group or a substituted or unsubstituted aryl group; R<sup>3</sup> represents a hydrogen atom, a substituted or unsubstituted alkyl group, a substituted or unsubstituted amino group, a substituted or unsubstituted alkoxy group, a substituted or unsubstituted aryloxy group, a substituted or unsubstituted alkoxy carbonyl group, a substituted or unsubstituted aryloxy carbonyl group, a substituted or unsubstituted aryl group, or a substituted or unsubstituted carbamoyl group; and R<sup>4</sup> represents a substituted or unsubstituted alkyl group, or a substituted or unsubstituted aryl group;



Formula (Y2) 30

wherein R<sup>5</sup> represents a substituted or unsubstituted alkyl group, or a substituted or unsubstituted alkenyl group, R<sup>6</sup> and R<sup>7</sup> each independently represent a substituted or unsubstituted alkyl group, R<sup>8</sup> represents a substituted or unsubstituted alkyl group, a substituted or unsubstituted aryl group, a substituted or unsubstituted alkoxy group, or a substituted or unsubstituted amino group, and R<sup>9</sup> represents a substituted or unsubstituted alkyl group, or a substituted or unsubstituted aryl group;



Formula (Y3)

wherein R<sup>10</sup> represents a hydrogen atom, or a substituted or unsubstituted alkyl group, R<sup>11</sup> represents a hydrogen atom or a halogen atom, and R<sup>12</sup> represents a substituted or unsubstituted alkoxy carbonyl group, a substituted or unsubstituted aryloxy carbonyl group, or a substituted or unsubstituted carbamoyl group;



Formula (Y4)

wherein the ring B represents a substituted or unsubstituted aryl group, or a substituted or unsubstituted aromatic heterocyclic group, R<sup>13</sup> represents a substituted or unsubstituted alkyl group, and R<sup>14</sup> represents a substituted or unsubstituted alkyl group, or a substituted or unsubstituted aryl group;



Formula (Y5)

wherein R<sup>15</sup>, R<sup>16</sup>, R<sup>17</sup> and R<sup>18</sup> each independently represent a substituted or unsubstituted alkyl group or a substituted or unsubstituted aryl group;



Formula (Y6)

wherein the rings C, D and E each independently represent a substituted or unsubstituted benzene ring;



Formula (Y7)

wherein the ring F represents a substituted or unsubstituted benzene ring; and R<sup>19</sup> and R<sup>20</sup> each independently represent a hydrogen atom, a substituted or unsubstituted alkyl group, a substituted or unsubstituted alkenyl group or a substituted or unsubstituted aryl group;



Formula (Y8)

wherein the ring G represents a substituted or unsubstituted benzene ring; and R<sup>21</sup> and R<sup>22</sup> each independently represent a hydrogen atom or a substituted or unsubstituted alkyl group; and

5



Formula (Y9)

6

resent a substituted or unsubstituted alkyl group, a substituted or unsubstituted alkenyl group or a substituted or unsubstituted aryl group;

5



Formula (M4)

wherein  $R^{23}$  represents a substituted or unsubstituted alkyl group or a substituted or unsubstituted alkenyl group.

(8) The heat-sensitive transfer sheet according to any one of items (1) to (7), wherein the above-described heat-sensitive transfer sheet contains at least one dye represented by any one of following formulae (M1) to (M8) set forth below:

Formula (M1)



15

wherein the ring H represents a substituted or unsubstituted benzene ring or a substituted or unsubstituted pyridine ring; and  $R^{24}$ ,  $R^{25}$ ,  $R^{26}$  and  $R^{27}$  each independently represent a substituted or unsubstituted alkyl group, a substituted or unsubstituted alkenyl group or a substituted or unsubstituted aryl group;

20

Formula (M5)



30

wherein  $R^{38}$  and  $R^{39}$  each independently represent a substituted or unsubstituted alkyl group, a substituted or unsubstituted aryl group, or a substituted or unsubstituted heterocyclic group, and  $R^{40}$  and  $R^{41}$  each independently represent a substituted or unsubstituted alkyl group, a substituted or unsubstituted alkenyl group, or a substituted or unsubstituted aryl group;

35



Formula (M2)

40

Formula (M6)



wherein the ring I represents a substituted or unsubstituted benzene ring or a substituted or unsubstituted pyridine ring; and  $R^{28}$ ,  $R^{29}$ ,  $R^{30}$  and  $R^{31}$  each independently represent a substituted or unsubstituted alkyl group, a substituted or unsubstituted alkenyl group or a substituted or unsubstituted aryl group;

50

wherein  $R^{42}$  is a substituted or unsubstituted aryloxy group,  $R^{43}$  is a hydrogen atom, or a substituted or unsubstituted aryloxy group, and  $R^{44}$  is a hydroxyl group, or a substituted or unsubstituted amino group;

55

Formula (M7)



Formula (M3)

60



wherein the ring J represents a substituted or unsubstituted benzene ring, and  $R^{32}$ ,  $R^{33}$  and  $R^{34}$  each independently rep-

65

wherein the ring L represents a substituted or unsubstituted benzene ring; and  $R^{45}$  and  $R^{46}$  each independently represent a hydrogen atom, a substituted or unsubstituted alkyl group, a substituted or unsubstituted alkenyl group or a substituted or unsubstituted aryl group; and



Formula (M8)



Formula (C3)

wherein the ring Q represents a substituted or unsubstituted benzene ring, R<sup>100</sup> represents a substituted or unsubstituted alkyl group, a substituted or unsubstituted aryl group, a substituted or unsubstituted alkoxy group, or a substituted or unsubstituted amino group, R<sup>101</sup> represents a substituted or unsubstituted alkyl group, or a substituted or unsubstituted aryl group, R<sup>102</sup> and R<sup>103</sup> each independently represent a hydrogen atom, a substituted or unsubstituted alkyl group, a substituted or unsubstituted alkenyl group, or a substituted or unsubstituted aryl group.

(9) The heat-sensitive transfer sheet according to any one of items (1) to (8), wherein the above-described heat-sensitive transfer sheet contains at least one dye represented by any one of following formulae (C1) to (C4) set forth below:



Formula (C1)

wherein the ring M represents a substituted or unsubstituted benzene ring, R<sup>47</sup> represents a hydrogen atom or a halogen atom, R<sup>48</sup> represents a substituted or unsubstituted alkyl group, R<sup>49</sup> represents a substituted or unsubstituted acylamino group or a substituted or unsubstituted alkoxy carbonylamino group, and R<sup>50</sup> and R<sup>51</sup> each independently represent a substituted or unsubstituted alkyl group, a substituted or unsubstituted alkenyl group or a substituted or unsubstituted aryl group;



Formula (C2)

wherein the ring N represents a substituted or unsubstituted benzene ring, R<sup>52</sup> represents a hydrogen atom, a substituted or unsubstituted acylamino group, a substituted or unsubstituted alkoxy carbonyl group, or a substituted or unsubstituted carbamoyl group, and R<sup>53</sup> and R<sup>54</sup> each independently represent a substituted or unsubstituted alkyl group, a substituted or unsubstituted alkenyl group, or a substituted or unsubstituted aryl group;

wherein R<sup>55</sup> and R<sup>56</sup> each independently represent an alkyl group, or a substituted or unsubstituted aryl group; and



Formula (C4)

25 wherein the ring O represents a substituted or unsubstituted benzene ring, and R<sup>57</sup> and R<sup>58</sup> each independently represent a substituted or unsubstituted alkyl group, a substituted or unsubstituted alkenyl group, or a substituted or unsubstituted aryl group.

30 (10) An image formation method in which images are formed in a state that the heat-sensitive transfer sheet according to any one of items (1) to (9) is superposed upon a heat-sensitive transfer image-receiving sheet having at least one dye-receiving layer on a support.

35 (11) The image formation method according to item (10), wherein the heat-sensitive transfer image-receiving sheet has at least one dye-receiving layer on a support, and further has at least one heat insulation layer containing hollow polymer particles and a hydrophilic polymer between the dye-receiving layer and the support.

40 The present invention will be explained in detail below.

1) Heat-Sensitive Transfer Sheet  
(Structure of the Heat-Sensitive Transfer Sheet (Ink Sheet))

The ink sheet is used to transfer a colorant (dye) from the ink sheet to a heat-sensitive transfer image-receiving sheet in the following manner: when a thermally transferred image is formed, the ink sheet is put onto the heat-sensitive transfer image-receiving sheet and then the sheets are heated from the ink sheet side thereof by means of a thermal printer head or the like. The ink sheet of the invention has a base film, a dye layer (heat-transferable layer) formed over one surface of the base film and containing a heat-transferable dye and a resin, and a heat-resistant lubricating layer formed over the other surface of the base film and containing an inorganic particle 45 and a resin. An easily-adhesive layer (primer layer) may be formed between the base film and the dye layer or between the base film and the heat-resistant lubricating layer.

In the invention, the inorganic particles contained in the heat-resistant lubricating layer need to have the following 50 requirements (I) to (III):

Requirement (I): the Mohs' hardness thereof ranges from 3 to 7;

Requirement (II): the mean particle size thereof ranges from 0.3 to 5  $\mu\text{m}$ ; and

Requirement (III): the ratio of the maximum width of each of the particles to the sphere equivalent diameter thereof is from 1.5 to 50.

The requirements (I) to (III) will be successively described hereinafter.

Requirement (I)

Mohs' hardness is a hardness originating from German mineralogist Friedrich Mohs' idea, and is a hardness digitized on the basis of the situation of scratches or injures of a substance when the substance is scratched by a standard substance. Substances listed up from a soft substance toward harder substances are successively specified as standard substances of indexes 1 to 10. Specifically, talc is specified as the standard substance 1; gypsum, 2; calcite, 3; fluorite, 4; apatite, 5; orthoclase, 6; quartz, 7; topaz, 8; corundum, 9; and diamond, 10. For example, in a case where a sample is scratched with fluorite, which is the standard substance 4, so that the sample is not injured but the sample is scratched with apatite, which is the standard substance 5, so that the sample is injured, this sample is harder than the index 4 and softer than the index 5. This is represented as a Mohs' hardness of "4 to 5", or "4.5". In a case where a sample is scratched with fluorite, which is the standard substance 4, so that not only the sample but also the fluorite are injured, the sample has the same hardness as the standard substance 4. This is represented as a Mohs' hardness of "4". Any numerical value of Mohs' hardness is a relative value but is not any absolute value.

If the Mohs' hardness is excessively small in the present invention, the heat-sensitive transfer sheet cannot be restrained from being deformed in high-speed printing. When Mohs' hardness is excessively large, the heat-sensitive transfer sheet injures a thermal printer head. In the invention, the Mohs' hardness is preferably from 3 to 6, more preferably from 3.5 to 5.5.

The inorganic particles having a Mohs' hardness of 3 to 7 may be known inorganic particles. Examples thereof include calcium carbonate (Mohs' hardness: 3), dolomite ( $MgCa(CO_3)_2$ ) (Mohs' hardness: 3.5-4), magnesium oxide (Mohs' hardness: 4), magnesium carbonate (Mohs' hardness: 3.5-4.5), and silica (Mohs' hardness: 7). Of these examples, preferable are magnesium oxide and magnesium carbonate, and more preferable is magnesium oxide.

Requirement (II)

In the invention, the mean particle size of the particles is a value obtained by the laser diffractive scattering method. The spatial distribution of the diffractive scattered light intensities obtained by radiating light to the particles is varied in accordance with the sizes of the particles. Thus, when the spatial distribution of the diffractive scattered light intensities is measured and analyzed, the distribution of the particle sizes can be obtained. Such a technique has been established as the laser diffractive scattering method. A device used for the measurement may be a commercially available product, such as SALD series manufactured by Shimadzu Corp. or LA series manufactured by Horiba Ltd. (tradename).

If the mean particle size is excessively small in the present invention, the heat-sensitive transfer sheet cannot be restrained from being deformed in high-speed printing and further the amount of materials adhering to a thermal printer head cannot be decreased. If the mean particle size is excessively large, the sheet is reversely deformed to a larger extent and simultaneously larger scratches and injures are given to a thermal printer head. Scratches and injures of a thermal printer head are equal to a matter that an insulating layer for protecting heat-generating electrode regions of the surface of the thermal printer head is injured and scratched. This makes the lifespan of the thermal printer head short. The mean particle size is preferably from 0.3 to 4.5  $\mu m$ , more preferably from 0.4 to 4  $\mu m$ .

Requirement (III)

The ratio of the maximum width of each of the inorganic particles to the sphere equivalent diameter thereof can be obtained from an observation of the particles with a scanning electron microscope, which is abbreviated to an "SEM". Specific steps therefor are as follows:

1. The inorganic particles are each observed with the SEM while the angle for the observation is varied. The shape, the length, and the thickness thereof are measured.

10 2. The particle volume is calculated out from the measured shape and size, and then the sphere equivalent diameter is obtained. The sphere equivalent diameter is the diameter of a sphere having a volume equal to the calculated-out particle volume. From the measured length and thickness, the maximum width of the particle is obtained. The maximum width of the particle is the maximum value out of lengths between any two points on the particle surface. When the inorganic particle is columnar, the maximum width corresponds to the height of the column. When the inorganic particle is a needle form, the maximum width corresponds to the length of the needle. When the inorganic particle is tabular, the maximum width corresponds to the largest width of the main plane(s).

25 3. The value of the ratio can be obtained by dividing the maximum width obtained about each of the particles by the sphere equivalent diameter. When the particulate form is spherical, the maximum width and the sphere equivalent diameter are equal to each other so that the ratio turns one. When the particulate form is cubic, the value of the ratio is about 1.4. As the particulate form is shifted more largely from 30 a sphere, the value of the ratio becomes larger.

When particles contain therein pores, the volume of the particles cannot be precisely calculated. In this case, however, the ratio is obtained by making calculation on the supposition that the particles have no pores.

35 4. If the ratio of the maximum width of each of the inorganic particles contained in the heat-resistant lubricating layer to the sphere equivalent diameter thereof is excessively small in the present invention, the effect of decreasing the amount of materials adhering to a thermal printer head is hardly produced and injures may be generated in the thermal printer head. If this ratio is excessively large, for example, about 70, which is obtained in a case where the inorganic particles are in a needle-form and the diameter and the length of the needles are 0.12  $\mu m$  and 88  $\mu m$ , respectively, the particles are 40 easily snapped by external stress. Thus, the inorganic particles are not easily incorporated into the heat-resistant lubricating layer in the state that the shape or form thereof is kept.

45 In connection with the ratio of the maximum width of each of the inorganic particles contained in the heat-resistant lubricating layer to the sphere equivalent diameter thereof, the ratio of the maximum width of any one selected from the inorganic particles contained in the heat-resistant lubricating layer to the sphere equivalent diameter thereof is varied in accordance with the selected particle. However, the ratio defined in the invention needs to range from 1.5 to 50 for 50 mass % or more of all the inorganic particles having a Mohs' hardness of 3 to 7, contained in the heat-resistant lubricating layer. This ratio ranges from 1.5 to 50 preferably for 80 mass % or more of all the inorganic particles having a Mohs' hardness of 3 to 7, contained in the heat-resistant lubricating layer, more preferably for 90 mass % or more thereof.

55 This ratio is preferably from 1.8 to 45, more preferably from 2 to 40.

60 Examples of the form of the inorganic particles wherein the ratio of the maximum width to the sphere equivalent diameter is from 1.5 to 50 in the invention include an indeterminate form; a columnar form; a needle form, which may be a spindle

## 11

form; and a tabular form. However, the form is not limited to these forms. The particulate form is preferably a needle form or tabular form, more preferably a tabular form. In a preferred embodiment, needle form inorganic particles and tabular inorganic particles may be used together.

In order to produce the advantageous effects of the invention, the ratio of the mass of the contained inorganic particles to the total coating mass of the heat-resistant lubricating layer needs to range from 0.001 to 5 mass %. If the ratio is excessively small, the advantageous effects are not produced. If the ratio is excessively large, injures are given to a thermal printer head. The ratio of the mass of the contained inorganic particles thereto is preferably from 0.005 to 3 mass %, more preferably from 0.01 to 2 mass %.

In the invention, the inorganic particles may be ones produced by a known method. When the inorganic particles are made of, for example, magnesium oxide, there are known: a method of firing a carbonate, a nitrate, a hydroxide and other salts of magnesium so as to be thermally decomposed; a method of subjecting magnesium to gas-phase oxidation; and other methods. In the firing, sintering or crystal growth is caused at the same time when the thermal decomposition is caused; thus, magnesium oxide in various forms can be produced in accordance with various conditions for the firing. In general, magnesium oxide resulting from firing at low temperature is called light burnt (calcined) magnesia, and magnesium oxide resulting from firing at high temperature is called heavy burnt magnesia (or dead burnt magnesia). An ingot obtained by melting magnesium oxide in a melting furnace such as an electric arc furnace and then solidifying the resultant is called electromelted magnesia. By pulverizing and/or classifying the resultant magnesium oxide particles, magnesium oxide particles having desired sizes can be obtained.

Inorganic particles contained as an impurity in a natural mineral may be used. JP-A-8-90945 states that dolomite ( $MgCa(CO_3)_2$ ), magnesite (made mainly of magnesium carbonate), silica and others that are contained as impurities in talc, which is a soft natural mineral, are incorporated together with talc. The Mohs' hardnesses of the impurities fall in the Mohs' hardness range defined in the invention, but the mean particle sizes thereof and the particulate forms thereof are not made clear. In general, talc particles obtained by selecting an appropriate mineral from natural minerals, pulverizing the selected mineral, and classifying the pulverized particles into a desired purity and desired sizes are used as a starting material. However, impurities in the talc are not easily set to desired sizes and a desired form. Moreover, dispersion in the size and the form between individual lots is not easily restrained. From this matter, the used inorganic particles are more preferably independently-produced particles than inorganic particles incorporated as impurities into the heat-resistant lubricating layer. In the case of magnesium oxide, magnesium oxide produced by firing is even more preferred from the viewpoint of productivity.

In the invention, it is particularly preferred that the amount of an impurity capable of forming inorganic particles having a Mohs' hardness of 3 or more, out of impurities contained in the inorganic particles, is small. In the case of magnesium oxide, the purity thereof is preferably 95 mass % or more, more preferably 98 mass % or more, most preferably 99 mass % or more. The total amount of calcium, silicon, iron, aluminum, chromium, cobalt, nickel, and copper as the impurities is preferably 2 mass % or less, even more preferably 1 mass % or less.

Besides the inorganic particles specified above, other additives may be used in the heat-resistant lubricating layer,

## 12

examples of the additive including a lubricant, a plasticizer, a stabilizer, a bulking agent, and a filler. In the following description, any inorganic compound having a Mohs' hardness less than 3 or more than 7 is not included in the inorganic compound specified above, and the above-specified mean particle size, particle form and the ratio by mass are not applied to the inorganic compound. When one or more of the inorganic compounds described below have a Mohs' hardness ranging from 3 to 7, the inorganic compound(s) may be used together so as to match the description of the above-mentioned inorganic particles.

Examples of the lubricant include fluorides such as calcium fluoride, barium fluoride, and graphite fluoride; sulfides such as molybdenum disulfide, tungsten disulfide, and iron sulfide; oxides such as silica, colloidal silica, lead oxide, alumina, and molybdenum oxide; solid lubricants each made of an inorganic compound such as graphite, mica, boron nitride, or a clay (such as talc, kaolin, or acid white clay); organic resins such as fluorine-contained resin and silicone resin; silicone oils; phosphate monoesters (a compound wherein one out of three  $—OH$  groups connected with a phosphorous atom in a single molecule of phosphoric acid is esterified) and phosphate diesters (a compound wherein two out of the  $—OH$  groups are esterified) and alkali metal salts thereof; phosphate triesters (a compound wherein all of the  $—OH$  groups are esterified); metal soaps such as polyvalent metal salts of an alkylcarboxylic acid (such as zinc stearate and lithium stearate), and polyvalent metal salts of a phosphate ester (such as zinc stearyl phosphate, and calcium polyoxyethylene tridecyl ether phosphate); various waxes such as polyethylene wax, and paraffin wax; and surfactants such as anionic surfactants, cationic surfactants, amphoteric surfactants, nonionic surfactants, and fluorine-contained surfactants. When a material originating from a natural mineral is used as a solid lubricant, an impurity having a Mohs' hardness 3 or more unfavorably damages the advantageous effects of the invention; thus, it is preferable that the amount of the impurity is as small as possible.

Of these additives, which may be used together, preferable are talc, kaolin, phosphate esters having at least one  $—OH$  group and alkali metal salts thereof, polyvalent metal salts of an alkylcarboxylic acid, and polyvalent metal salts of a phosphate ester.

In the present invention, as an alchol section of the molecule of the above phosphate monoesters, diesters or tiesters, it is preferable to employ that of an aliphatic alchol having 10 to 20 carbon atoms. Further, metal salts of the alkylcarboxylic acid above-stated is preferably an alkylcarboxylic acid having 10 to 20 carbon atoms for its carboxylic acid section.

Further, combination of the above phosphate monoesters, diesters or tiesters and the above metal salts of the alkylcarboxylic acid is the most preferable, in the view of effect of the present invention.

Some ester surfactants have acid groups. As a result, when a large calorie is given thereto from a thermal head, the esters may decompose and further the pH of the backside layer may be lowered to corrode and abrade the thermal head largely. Examples of a method to be adopted against this problem include a method of using a neutralized ester surfactant, and a method of using a neutralizing agent such as magnesium hydroxide.

Other examples of the additives include higher aliphatic alcohols, organopolysiloxanes, and organic carboxylic acids.

The heat-resistant lubricating layer needs to contain a resin. The resin may be a known resin. Examples thereof include cellulose resins such as ethylcellulose, hydroxycellulose, hydroxypropylcellulose, methylcellulose, cellulose

acetate, cellulose acetate butyrate, cellulose acetate propionate, and nitrocellulose; vinyl resins such as polyvinyl alcohol resin, polyvinyl acetate resin, polyvinyl butyral, polyvinyl acetal, polyvinyl acetoacetal resin, vinyl chloride-vinyl acetal copolymer and polyvinyl pyrrolidone; (meth)acrylic resins such as methyl polymethacrylate, ethyl polyacrylate, polyacrylamide, and acrylonitrile-styrene copolymer; other resins such as polyamide resin, polyimide resin, polyamide-imide resin, polyvinyl toluene resin, coumarone indene resin, polyester resin, polyurethane resin, polyether resin, polybutadiene resin, polycarbonate resin, chlorinated polyolefin resin, fluorine-contained resin, epoxy resin, phenol resin, silicone resin, silicone-modified or fluorine-modified urethane, and other natural or synthetic resins. These may be used alone or in a mixture form.

The resin may be crosslinked by radiating ultraviolet rays or an electron beam thereto in order to make the heat resistance high. A crosslinking agent may be used to crosslink the resin by aid of heating. At this time, a catalyst may be added thereto. Examples of the crosslinking agent include isocyanate based agents (such as polyisocyanate, and a cyclic trimer of polyisocyanate), and metal-containing agents (such as titanium tetrabutylate, zirconium tetrabutylate, and aluminum triisopropionate). Examples of the resin with which these crosslinking agents are each caused to react include polyvinyl acetal, polyvinyl butyral, polyester polyol, alkyd polyol, and silicone compounds containing, in side chains thereof, amino groups.

The heat-resistant lubricating layer is formed by adding the essential components and optional additives to the binder, examples of which have been described above, dissolving or dispersing the resultant into a solvent to prepare a coating solution, and then painting the coating solution by a known method such as gravure coating, roll coating, blade coating or wire bar coating. The film thickness of the heat-resistant lubricating layer is preferably from 0.1 to 3  $\mu\text{m}$ , more preferably from 0.2 to 2  $\mu\text{m}$ .

(Base Film)

As the base film, any one of known materials can be used, so far as such the material has both a heat resistance and a mechanical strength necessary to the requirements for the support. Specific examples of preferable base films include thin papers such as a glassine paper, a condenser paper, and a paraffin paper; polyesters having high resistance to heat such as polyethyleneterephthalate, polyethylenenaphthalate, polybutyleneterephthalate, polyphenylene sulfide, polyetherketone, and polyethersulfone; stretched or unstretched films of plastics such as polypropylene, polycarbonate, cellulose acetate, polyethylene derivatives, poly(vinyl chloride), poly(vinylidene chloride), polystyrene, polyamide, polyimide, polymethylpentene, and ionomers; and laminates of these materials. Of these materials, polyester films are especially preferred. Stretched polyester films are most preferred. A thickness of the base film can be properly determined in accordance with the material of the base film so that the mechanical strength and the heat resistance become optimum. Specifically, it is preferred to use a support having a thickness of about 1  $\mu\text{m}$  to about 30  $\mu\text{m}$ , more preferably from about 1  $\mu\text{m}$  to 20  $\mu\text{m}$ , and further preferably from about 3  $\mu\text{m}$  to about 10  $\mu\text{m}$ .

The dye layer containing a heat-transferable dye (hereinafter also referred to as the heat-sensitive transfer layer or the heat transfer layer) can be formed by painting a dye ink.

(Dye Layer)

In the dye layer in the invention, preferably, dye (sub)layers in individual colors of yellow, magenta and cyan, and an optional dye (sub)layer in black are repeatedly painted onto a

single support in area order in such a manner that the colors are divided from each other. An example of the dye layer is an embodiment wherein dye (sub)layers in individual colors of yellow, magenta and cyan are painted onto a single support along the long axial direction thereof in area order, correspondingly to the area of the recording surface of the above-mentioned heat-sensitive transfer image-receiving sheet, in such a manner that the colors are divided from each other. Another example thereof is an embodiment wherein not only the three (sub)layers but also a dye (sub)layer in black and/or a transferable protective layer are painted in such a manner that these (sub)layers are divided from each other. This embodiment is preferred.

In the case of adopting such an embodiment, it is preferred to give marks to the heat-sensitive transfer sheet in order to inform the printer about starting point of the individual colors. Such painting repeated in area order makes it possible that a single heat-sensitive transfer sheet is used to form an image on the basis of transfer of dyes and further laminate a protective layer on the image.

In the invention, however, the manner in which the dye layer is formed is not limited to the above-mentioned manners. A sublimation heat-transferable ink layer and a heat-melt transferable ink layer may be together formed. A dye in a color other than yellow, magenta, cyan and black is formed, or other modifications may be made. The form of the heat-sensitive transfer sheet including the dye layer may be a longitudinal form, or a one-piece form.

The dye layer may have a mono-layered structure or a multi-layered structure. In the case of the multi-layered structure, the individual layers constituting the dye layer may be the same or different in composition.

(Dye Ink)

The dye layer contains at least a sublimation type dye and a binder resin. It is a preferable embodiment of the present invention that the ink may contain organic or inorganic finely divided powder, waxes, silicone resins, and fluorine-containing organic compounds, in accordance with necessity.

Each dye in the dye layer is preferably contained in an amount of 10 to 90 mass % of the dye layer, preferably in that of 20 to 80 mass % thereof.

The coating of the dye layer (i.e., the painting of a coating solution for the dye layer) is performed by an ordinary method such as roll coating, bar coating, gravure coating, or gravure reverse coating. The coating amount of the dye layer is preferably from 0.1 to 2.0  $\text{g}/\text{m}^2$ , more preferably from 0.2 to 1.2  $\text{g}/\text{m}^2$  (the amount is a numerical value converted to the solid content in the layer; any coating amount in the following description is a numerical value converted to the solid content unless otherwise specified). The film thickness of the dye layer is preferably from 0.1 to 2.0  $\mu\text{m}$ , more preferably from 0.2 to 1.2  $\mu\text{m}$ .

(The Dyes)

The dyes contained in the dye layer in the present invention must be the dyes that are able to diffuse by heat and able to be incorporated in a heat-sensitive transfer sheet, and able to transfer by heat from the heat-sensitive transfer sheet to an image-receiving sheet. As the dyes that are used for the heat-sensitive transfer sheet, ordinarily used dyes or known dyes can be effectively used.

Preferable examples of the dyes that are used in the present invention include diarylmethane-series dyes, triarylmethane-series dyes, thiazole-series dyes, methine-series dyes such as merocyanine; azomethine-series dyes typically exemplified by indoaniline, acetophenoneazomethine, pyrazoloazomethine, imidazole azomethine, imidazo azomethine, and pyridone azomethine; xanthene-series dyes; oxazine-series dyes;

## 15

cyanomethylene-series dyes typically exemplified by dicyanostyrene, and tricyanostyrene; thiazine-series dyes; azine-series dyes; acridine-series dyes; benzene azo-series dyes; azo-series dyes such as pyridone azo, thiophene azo, isothiazole azo, pyrrol azo, pyralazo, imidazole azo, thiadiazole azo, triazole azo, and disazo; spiropyran-series dyes; indolino-spiropyran-series dyes; fluoran-series dyes; rhodaminelactam-series dyes; naphthoquinone-series dyes; anthraquinone-series dyes; and quinophthalon-series dyes.

Specific examples of the yellow dyes include Disperse Yellow 231, Disperse Yellow 201 and Solvent Yellow 93. Specific examples of the magenta dyes include Disperse Violet 26, Disperse Red 60, and Solvent Red 19. Specific examples of the cyan dyes include Solvent Blue 63, Solvent Blue 36, Disperse Blue 354 and Disperse Blue 35. As a matter of course, it is also possible to use suitable dyes other than these dyes as exemplified above.

Further, dyes each having a different hue from each other as described above may be arbitrarily combined together. For instance, a black hue can be obtained from a combination of dyes.

In the present invention, dyes represented by any one of formulae (Y1) to (Y9), formulae (M1) to (M8), and formulae (C1) to (C4) set forth below are preferably used.

These dyes are explained in detail below.



Formula (Y1)

In the formula (Y1), the ring A represents a substituted or unsubstituted benzene ring; R<sup>1</sup> and R<sup>2</sup> each independently represent a hydrogen atom, a substituted or unsubstituted alkyl group, a substituted or unsubstituted alkenyl group or a substituted or unsubstituted aryl group; R<sup>3</sup> represents a hydrogen atom, a substituted or unsubstituted alkyl group, a substituted or unsubstituted amino group, a substituted or unsubstituted alkoxy group, a substituted or unsubstituted aryloxy group, a substituted or unsubstituted alkoxy carbonyl group, a substituted or unsubstituted aryloxycarbonyl group, a substituted or unsubstituted aryl group, or a substituted or unsubstituted carbamoyl group; and R<sup>4</sup> represents a substituted or unsubstituted alkyl group, or a substituted or unsubstituted aryl group.

Examples of the substituent by which each of the ring A and the groups R<sup>1</sup>, R<sup>2</sup>, R<sup>3</sup> and R<sup>4</sup> may be substituted include halogen atoms, unsaturated aliphatic groups, aryl groups, heterocyclic groups, aliphatic oxy groups (typically, alkoxy groups), acyloxy groups, carbamoyloxy groups, aliphatic oxycarbonyloxy groups (typically, alkoxy carbonyloxy groups), aryloxycarbonyl groups, amino groups, acylamino groups, aminocarbonylamino groups, aliphatic oxycarbonylamino groups (typically, alkoxy carbonylamino groups), sulfamoylamino groups, aliphatic (typically, alkyl) or arylsulfonylamino groups, aliphatic thio groups (typically, alkylthio groups), sulfamoyl groups, aliphatic (typically, alkyl) or arylsulfinyl groups, aliphatic (typically, alkyl) or arylsulfonyl groups, acyl groups, aryloxycarbonyl groups, aliphatic oxy-carbonyl groups (typically, alkoxy carbonyl groups), carbam-

## 16

oyl groups, aryl or heterocyclic azo groups, imide groups, a hydroxy group, a cyano group, a nitro group, a sulfo group, and a carboxyl group.

These groups may each further have a substituent. Examples of the substituent include the above-mentioned substituents.

Examples of a preferred combination of the ring A and groups R<sup>1</sup> to R<sup>4</sup> in the dye represented by the formula (Y1) include combinations wherein the ring A is a substituted or unsubstituted benzene ring, R<sup>1</sup> is a substituted or unsubstituted alkyl group having 1 to 8 carbon atoms, an allyl group, or a substituted or unsubstituted aryl group having 6 to 10 carbon atoms, R<sup>2</sup> is a substituted or unsubstituted alkyl group having 1 to 8 carbon atoms, an allyl group, or a substituted or unsubstituted aryl group having 6 to 10 carbon atoms, R<sup>3</sup> is a substituted or unsubstituted amino group, or a substituted or unsubstituted alkoxy group, and R<sup>4</sup> is a substituted or unsubstituted alkyl group having 1 to 8 carbon atoms, or a substituted or unsubstituted aryl group having 6 to 10 carbon atoms.

In more preferred combinations thereof, the ring A is a substituted or unsubstituted benzene ring, R<sup>1</sup> is a substituted or unsubstituted alkyl group having 1 to 6 carbon atoms, an allyl group, or a substituted or unsubstituted phenyl group, R<sup>2</sup> is a substituted or unsubstituted alkyl group having 1 to 6 carbon atoms, an allyl group, or a substituted or unsubstituted phenyl group, R<sup>3</sup> is a substituted or unsubstituted amino group, or a substituted or unsubstituted alkoxy group, and R<sup>4</sup> is a substituted or unsubstituted alkyl group having 1 to 6 carbon atoms, or a substituted or unsubstituted phenyl group.

In the most preferred combinations thereof, the ring A is a benzene ring substituted by a methyl group or a chlorine atom, or an unsubstituted benzene ring, R<sup>1</sup> is a substituted or unsubstituted alkyl group having 1 to 4 carbon atoms, or an allyl group, R<sup>2</sup> is a substituted or unsubstituted alkyl group having 1 to 4 carbon atoms, or an allyl group, R<sup>3</sup> is a substituted or unsubstituted amino group, or a substituted or unsubstituted alkoxy group, and R<sup>4</sup> is a substituted or unsubstituted phenyl group.



Formula (Y2)

In the formula (Y2), R<sup>5</sup> represents a substituted or unsubstituted alkyl group, or a substituted or unsubstituted alkenyl group, R<sup>6</sup> and R<sup>7</sup> each independently represent a substituted or unsubstituted alkyl group, R<sup>8</sup> represents a substituted or unsubstituted alkyl group, a substituted or unsubstituted aryl group, a substituted or unsubstituted alkoxy group, or a substituted or unsubstituted amino group, and R<sup>9</sup> represents a substituted or unsubstituted alkyl group, or a substituted or unsubstituted aryl group.

Each of the groups represented by R<sup>5</sup>, R<sup>6</sup>, R<sup>7</sup>, R<sup>8</sup> and R<sup>9</sup> may further have a substituent. Examples of a substituent by which each of the groups of R<sup>5</sup>, R<sup>6</sup>, R<sup>7</sup>, R<sup>8</sup> and R<sup>9</sup> may be substituted include the same substituents as each of the ring A and the substituents R<sup>1</sup> to R<sup>4</sup> in the formula (Y1) may have.

Examples of a preferred combination of the groups R<sup>5</sup> to R<sup>9</sup> in the dye represented by the formula (Y2) include combinations wherein R<sup>5</sup> is a substituted or unsubstituted alkyl group having 1 to 8 carbon atoms, or an allyl group, R<sup>6</sup> is a

17

substituted or unsubstituted alkyl group having 1 to 8 carbon atoms, R<sup>7</sup> is a substituted or unsubstituted alkyl group having 1 to 8 carbon atoms, R<sup>8</sup> is a substituted or unsubstituted alkyl group having 1 to 8 carbon atoms, a substituted or unsubstituted aryl group having 6 to 10 carbon atoms, a substituted or unsubstituted alkoxy group having 1 to 8 carbon atoms, or a substituted or unsubstituted amino group, and R<sup>9</sup> represents a substituted or unsubstituted alkyl group having 1 to 8 carbon atoms, or a substituted or unsubstituted aryl group having 6 to 10 carbon atoms.

In more preferred combinations thereof, R<sup>5</sup> is a substituted or unsubstituted alkyl group having 1 to 6 carbon atoms, or an allyl group, R<sup>6</sup> is a substituted or unsubstituted alkyl group having 1 to 6 carbon atoms, R<sup>7</sup> is a substituted or unsubstituted alkyl group having 1 to 6 carbon atoms, R<sup>8</sup> is a substituted or unsubstituted alkyl group having 1 to 6 carbon atoms, a substituted or unsubstituted phenyl group, a substituted or unsubstituted alkoxy group having 1 to 6 carbon atoms, or a substituted or unsubstituted amino group, and R<sup>9</sup> represents a substituted or unsubstituted alkyl group having 1 to 6 carbon atoms, or a substituted or unsubstituted phenyl group.

In the most preferred combinations thereof, R<sup>5</sup> is an unsubstituted alkyl group having 1 to 4 carbon atoms, R<sup>6</sup> is an unsubstituted alkyl group having 1 to 4 carbon atoms, R<sup>7</sup> is an unsubstituted alkyl group having 1 to 4 carbon atoms, R<sup>8</sup> is a methoxy, ethoxy, or dimethylamino group, and R<sup>9</sup> is an unsubstituted phenyl group.



Formula (Y3)

In the formula (Y3), R<sup>10</sup> represents a hydrogen atom, or a substituted or unsubstituted alkyl group, R<sup>11</sup> represents a hydrogen atom or a halogen atom, and R<sup>12</sup> represents a substituted or unsubstituted alkoxy carbonyl group, a substituted or unsubstituted aryloxy carbonyl group, or a substituted or unsubstituted carbamoyl group.

Each of the groups represented by R<sup>10</sup> and R<sup>12</sup> may further have a substituent. Examples of a substituent by which each of the groups of R<sup>10</sup> and R<sup>12</sup> may be substituted include the same substituents as each of the ring A and the substituents R<sup>1</sup> to R<sup>4</sup> in the formula (Y1) may have.

Examples of a preferred combination of the groups R<sup>10</sup> to R<sup>12</sup> in the dye represented by the formula (Y3) include combinations wherein R<sup>10</sup> is a hydrogen atom or a substituted or unsubstituted alkyl group having 1 to 8 carbon atoms, R<sup>11</sup> is a hydrogen atom, a chlorine atom, or a bromine atom, and R<sup>12</sup> is an unsubstituted alkoxy carbonyl group, an unsubstituted aryloxy carbonyl group, or a substituted or unsubstituted carbamoyl group.

In more preferred combinations thereof, R<sup>10</sup> is a hydrogen atom or a substituted or unsubstituted alkyl group having 1 to 6 carbon atoms, R<sup>11</sup> is a hydrogen atom or a bromine atom, and R<sup>12</sup> is an unsubstituted alkoxy carbonyl group having 2 to 10 carbon atoms, or a dialkyl carbamoyl group having 2 to 12 carbon atoms.

18

In the most preferred combinations thereof, R<sup>10</sup> is a hydrogen atom or an unsubstituted alkyl group having 2 to 4 carbon atoms, R<sup>11</sup> is a hydrogen atom, and R<sup>12</sup> is a dialkyl carbamoyl group having 2 to 10 carbon atoms.



Formula (Y4)

In the formula (Y4), the ring B represents a substituted or unsubstituted aryl group, or a substituted or unsubstituted aromatic heterocyclic group, R<sup>13</sup> represents a substituted or unsubstituted alkyl group, and R<sup>14</sup> represents a substituted or unsubstituted alkyl group, or a substituted or unsubstituted aryl group.

Each of the ring B and the groups represented by R<sup>13</sup> and R<sup>14</sup> may further have a substituent. Examples of a substituent by which each of the ring B and the groups of R<sup>13</sup> and R<sup>14</sup> may be substituted include the same substituents as each of the ring A and the substituents R<sup>1</sup> to R<sup>4</sup> in the formula (Y1) may have.

Examples of a preferred combination of the ring B and the groups R<sup>13</sup> and R<sup>14</sup> in the dye represented by the formula (Y4) include combinations wherein the ring B is a substituted or unsubstituted aryl group having 6 to 10 carbon atoms, a substituted or unsubstituted pyrazolyl group, or a substituted or unsubstituted thiadiazolyl group, R<sup>13</sup> is a substituted or unsubstituted alkyl group having 1 to 8 carbon atoms, and R<sup>14</sup> is a substituted or unsubstituted alkyl group having 1 to 8 carbon atoms, or a substituted or unsubstituted aryl group having 6 to 10 carbon atoms.

In more preferred combinations thereof, the ring B is a substituted or unsubstituted phenyl group, or a substituted or unsubstituted 1,3,4-thiadiazolyl group, R<sup>13</sup> is a substituted or unsubstituted alkyl group having 1 to 6 carbon atoms, and R<sup>14</sup> is a substituted or unsubstituted alkyl group having 1 to 6 carbon atoms, or a substituted or unsubstituted phenyl group.

In the most preferred combinations thereof, the ring B is a 4-nitrophenyl group, or a 1,3,4-thiadiazolyl group having a thioalkyl group having 1 to 6 carbon atoms as a substituent, R<sup>13</sup> is an unsubstituted alkyl group having 1 to 4 carbon atoms, and R<sup>14</sup> is an unsubstituted alkyl group having 1 to 4 carbon atoms, or a substituted or unsubstituted phenyl group.



Formula (Y5)

In the formula (Y5), R<sup>15</sup>, R<sup>16</sup>, R<sup>17</sup> and R<sup>18</sup> each independently represent a substituted or unsubstituted alkyl group or a substituted or unsubstituted aryl group.

Each of the groups represented by R<sup>15</sup>, R<sup>16</sup>, R<sup>17</sup> and R<sup>18</sup> may further have a substituent. Examples of a substituent by which each of the groups of R<sup>15</sup>, R<sup>16</sup>, R<sup>17</sup> and R<sup>18</sup> may be

19

substituted include the same substituents as each of the ring A and the substituents R<sup>1</sup> to R<sup>4</sup> in the formula (Y1) may have.

Examples of a preferred combination of the substituents R<sup>15</sup> to R<sup>18</sup> in a dye represented by the formula (Y5) include combinations wherein R<sup>15</sup> is a substituted or unsubstituted alkyl group having 1 to 8 carbon atoms or a substituted or unsubstituted aryl group having 6 to 10 carbon atoms, R<sup>16</sup> is a substituted or unsubstituted alkyl group having 1 to 8 carbon atoms or a substituted or unsubstituted aryl group having 6 to 10 carbon atoms, R<sup>17</sup> is a substituted or unsubstituted alkyl group having 1 to 8 carbon atoms or a substituted or unsubstituted aryl group having 6 to 10 carbon atoms, and R<sup>18</sup> is a substituted or unsubstituted alkyl group having 1 to 8 carbon atoms or a substituted or unsubstituted aryl group having 6 to 10 carbon atoms.

In more preferred combinations of the substituents R<sup>15</sup> to R<sup>18</sup>, R<sup>15</sup> is a substituted or unsubstituted alkyl group having 1 to 6 carbon atoms, R<sup>16</sup> is a substituted or unsubstituted alkyl group having 1 to 6 carbon atoms, R<sup>17</sup> is a substituted or unsubstituted phenyl group, and R<sup>18</sup> is a substituted or unsubstituted phenyl group.

In the most preferred combinations thereof, R<sup>15</sup> is a substituted or unsubstituted alkyl group having 1 to 4 carbon atoms, R<sup>16</sup> is a substituted or unsubstituted alkyl group having 1 to 4 carbon atoms, R<sup>17</sup> is an unsubstituted phenyl group, and R<sup>18</sup> is an unsubstituted phenyl group.

Formula (Y6)



In the formula (Y6), the rings C, D and E each independently represent a substituted or unsubstituted benzene ring.

Each of the rings C, D and E may further have a substituent. Examples of a substituent by which each of the rings C, D and E may be substituted include the same substituents as each of the ring A and the substituents R<sup>1</sup> to R<sup>4</sup> in the formula (Y1) may have.

The ring C is preferably a benzene ring substituted by an alkyl group having 1 to 8 carbon atoms, a benzene ring substituted by an alkoxy group having 1 to 8 carbon atoms, a benzene ring substituted by a hydroxyl group, or an unsubstituted benzene ring, more preferably a benzene ring substituted by an alkyl group having 1 to 6 carbon atoms, a benzene ring substituted by an alkoxy group having 1 to 6 carbon atoms, or a benzene ring substituted by a hydroxyl group, most preferably a benzene ring substituted by an alkyl group having 1 to 4 carbon atoms, or a benzene ring substituted by an alkoxy group having 1 to 4 carbon atoms.

The ring D is preferably a benzene ring substituted by an alkyl group having 1 to 8 carbon atoms, or an unsubstituted benzene ring, more preferably a benzene ring substituted by an alkyl group having 1 to 6 carbon atoms, or an unsubstituted benzene ring, most preferably a benzene ring substituted by an alkyl group having 1 to 4 carbon atoms, or an unsubstituted benzene ring.

The ring E is preferably a benzene ring substituted by a hydroxyl group and an alkyl group having 1 to 8 carbon atoms, or a benzene ring substituted by a hydroxyl group and an alkoxy group having 1 to 8 carbon atoms, more preferably a benzene ring substituted by a hydroxyl group and an alkyl group having 1 to 6 carbon atoms, or a benzene ring substituted by a hydroxyl group and an alkoxy group having 1 to 6 carbon atoms, most preferably a benzene ring substituted by

20

a hydroxyl group and an alkyl group having 1 to 4 carbon atoms, or a benzene ring substituted by a hydroxyl group and an alkoxy group having 1 to 4 carbon atoms.



Formula (Y7)

In the formula (Y7), the ring F represents a substituted or unsubstituted benzene ring; and R<sup>19</sup> and R<sup>20</sup> each independently represent a hydrogen atom, a substituted or unsubstituted alkyl group, a substituted or unsubstituted alkenyl group or a substituted or unsubstituted aryl group.

Each of the ring F and the groups represented by R<sup>19</sup> and R<sup>20</sup> may further have a substituent. Examples of a substituent by which each of the ring F and the groups of R<sup>19</sup> and R<sup>20</sup> may be substituted include the same substituents as each of the ring A and the substituents R<sup>1</sup> to R<sup>4</sup> in the formula (Y1) may have.

Examples of a preferred combination of the ring F and the substituents R<sup>19</sup> and R<sup>20</sup> in a dye represented by the formula (Y7) include combinations wherein the ring F is an unsubstituted benzene ring, R<sup>19</sup> is a substituted or unsubstituted alkyl group having 1 to 8 carbon atoms, an allyl group or a substituted or unsubstituted aryl group having 6 to 10 carbon atoms, and R<sup>20</sup> is a substituted or unsubstituted alkyl group having 1 to 8 carbon atoms, an allyl group or a substituted or unsubstituted aryl group having 6 to 10 carbon atoms.

In more preferred combinations of the ring F and the substituents R<sup>19</sup> and R<sup>20</sup>, the ring F is a substituted or unsubstituted benzene ring, R<sup>19</sup> is a substituted or unsubstituted alkyl group having 1 to 6 carbon atoms, an allyl group or a substituted or unsubstituted phenyl group, and R<sup>20</sup> is a substituted or unsubstituted alkyl group having 1 to 6 carbon atoms, an allyl group or a substituted or unsubstituted phenyl group.

In the most preferred combinations thereof, the ring F is a benzene ring substituted by a methyl group, R<sup>19</sup> is an unsubstituted alkyl group having 1 to 4 carbon atoms, and R<sup>20</sup> is a substituted alkyl group having 1 to 4 carbon atoms.



Formula (Y8)

In the formula (Y8), the ring G represents a substituted or unsubstituted benzene ring; and R<sup>21</sup> and R<sup>22</sup> each independently represent a hydrogen atom or a substituted or unsubstituted alkyl group.

Each of the ring G and the groups represented by R<sup>21</sup> and R<sup>22</sup> may further have a substituent. Examples of a substituent by which each of the ring G and the groups of R<sup>21</sup> and R<sup>22</sup> may be substituted include the same substituents as each of the ring A and the substituents R<sup>1</sup> to R<sup>4</sup> in the formula (Y1) may have.

Examples of a preferred combination of the ring G and the substituents R<sup>21</sup> and R<sup>22</sup> include combinations wherein the ring G is a benzene ring having a substituent(s), R<sup>21</sup> is a

## 21

substituted or unsubstituted alkyl group having 1 to 8 carbon atoms, and  $R^{22}$  is a substituted or unsubstituted alkyl group having 1 to 8 carbon atoms.

In more preferred combinations thereof, the ring G is a benzene ring substituted by a substituted or unsubstituted alkoxy carbonyl group,  $R^{21}$  is a substituted or unsubstituted alkyl group having 1 to 6 carbon atoms, and  $R^{22}$  is a substituted or unsubstituted alkyl group having 1 to 6 carbon atoms.

In the most preferred combinations thereof, the ring G is a benzene ring substituted by a substituted or unsubstituted alkoxy carbonyl group,  $R^{21}$  is a substituted or unsubstituted alkyl group having 1 to 4 carbon atoms, and  $R^{22}$  is a substituted or unsubstituted alkyl group having 1 to 4 carbon atoms.

Formula (Y9)



In the formula (Y9),  $R^{23}$  represents a substituted or unsubstituted alkyl group or a substituted or unsubstituted alkenyl group.

The group represented by  $R^{23}$  may further have a substituent. Examples of a substituent by which the group of  $R^{23}$  may be substituted include the same substituents as each of the ring A and the substituents  $R^1$  to  $R^4$  in the formula (Y1) may have.

$R^{23}$  is preferably a substituted or unsubstituted alkyl group having 1 to 8 carbon atoms or an allyl group, more preferably a substituted or unsubstituted alkyl group having 1 to 6 carbon atoms or an allyl group, and most preferably a substituted or unsubstituted alkyl group having 1 to 4 carbon atoms or an allyl group.

Formula (M1)



In the formula (M1), the ring H represents a substituted or unsubstituted benzene ring or a substituted or unsubstituted pyridine ring; and  $R^{24}$ ,  $R^{25}$ ,  $R^{26}$  and  $R^{27}$  each independently represent a substituted or unsubstituted alkyl group, a substituted or unsubstituted alkenyl group or a substituted or unsubstituted aryl group.

Each of the ring H and the groups represented by  $R^{24}$ ,  $R^{25}$ ,  $R^{26}$  and  $R^{27}$  may further have a substituent. Examples of a substituent by which each of the ring H and the groups of  $R^{24}$ ,  $R^{25}$ ,  $R^{26}$  and  $R^{27}$  may be substituted include the same substituents as each of the ring A and the substituents  $R^1$  to  $R^4$  in the formula (Y1) may have.

Examples of a preferred combination of the ring H and the substituents  $R^{24}$  to  $R^{27}$  in a dye represented by the formula (M1) include combinations wherein the ring H is an unsub-

## 22

stituted benzene ring,  $R^{24}$  is a substituted or unsubstituted alkyl group having 1 to 8 carbon atoms or a substituted or unsubstituted aryl group having 6 to 10 carbon atoms,  $R^{25}$  is a substituted or unsubstituted alkyl group having 1 to 8 carbon atoms or a substituted or unsubstituted aryl group having 6 to 10 carbon atoms,  $R^{26}$  is a substituted or unsubstituted alkyl group having 1 to 8 carbon atoms or an allyl group, and  $R^{27}$  is a substituted or unsubstituted alkyl group having 1 to 8 carbon atoms or an allyl group.

In more preferred combinations of the ring H and the substituents  $R^{24}$  to  $R^{27}$ , the ring H is an unsubstituted benzene ring,  $R^{24}$  is a substituted or unsubstituted phenyl group,  $R^{25}$  is a substituted or unsubstituted alkyl group having 1 to 8 carbon atoms,  $R^{26}$  is a substituted or unsubstituted alkyl group having 1 to 6 carbon atoms, and  $R^{27}$  is a substituted or unsubstituted alkyl group having 1 to 6 carbon atoms.

In the most preferred combinations, the ring H is an unsubstituted benzene ring,  $R^{24}$  is a 2-chlorophenyl group,  $R^{25}$  is a substituted or unsubstituted alkyl group having 1 to 4 carbon atoms,  $R^{26}$  is a substituted or unsubstituted alkyl group having 1 to 4 carbon atoms, and  $R^{27}$  is a substituted or unsubstituted alkyl group having 1 to 4 carbon atoms.



In the formula (M2), the ring I represents a substituted or unsubstituted benzene ring or a substituted or unsubstituted pyridine ring; and  $R^{28}$ ,  $R^{29}$ ,  $R^{30}$  and  $R^{31}$  each independently represent a substituted or unsubstituted alkyl group, a substituted or unsubstituted alkenyl group or a substituted or unsubstituted aryl group.

Each of the ring I and the groups represented by  $R^{28}$ ,  $R^{29}$ ,  $R^{30}$  and  $R^{31}$  may further have a substituent. Examples of a substituent by which each of the ring I and the groups of  $R^{28}$ ,  $R^{29}$ ,  $R^{30}$  and  $R^{31}$  may be substituted include the same substituents as each of the ring A and the substituents  $R^1$  to  $R^4$  in the formula (Y1) may have.

Examples of a preferred combination of the ring I and the substituents  $R^{28}$  to  $R^{31}$  in a dye represented by the formula (M2) include combinations wherein the ring I is a substituted or unsubstituted pyridine ring or an unsubstituted benzene ring,  $R^{28}$  is a substituted or unsubstituted alkyl group having 1 to 8 carbon atoms or a substituted or unsubstituted aryl group having 6 to 10 carbon atoms,  $R^{29}$  is a substituted or unsubstituted alkyl group having 1 to 8 carbon atoms or a substituted or unsubstituted aryl group having 6 to 10 carbon atoms,  $R^{30}$  is a substituted or unsubstituted alkyl group having 1 to 8 carbon atoms or an allyl group, and  $R^{31}$  is a substituted or unsubstituted alkyl group having 1 to 8 carbon atoms or an allyl group.

In more preferred combinations of the ring I and the substituents  $R^{28}$  to  $R^{31}$ , the ring I is a substituted or unsubstituted pyridine ring or an unsubstituted benzene ring,  $R^{28}$  is a substituted or unsubstituted alkyl group having 1 to 6 carbon atoms,  $R^{29}$  is a substituted or unsubstituted alkyl group having 1 to 6 carbon atoms,  $R^{30}$  is a substituted or unsubstituted

alkyl group having 1 to 6 carbon atoms, and  $R^{31}$  is a substituted or unsubstituted alkyl group having 1 to 6 carbon atoms.

In the most preferred combinations thereof, the ring I is a substituted or unsubstituted pyridine ring or an unsubstituted benzene ring,  $R^{28}$  is a substituted or unsubstituted alkyl group having 1 to 4 carbon atoms,  $R^{29}$  is a substituted or unsubstituted alkyl group having 1 to 4 carbon atoms,  $R^{30}$  is a substituted or unsubstituted alkyl group having 1 to 4 carbon atoms, and  $R^{31}$  is a substituted or unsubstituted alkyl group having 1 to 4 carbon atoms.



In the formula (M3), the ring J represents a substituted or unsubstituted benzene ring, and  $R^{32}$ ,  $R^{33}$  and  $R^{34}$  each independently represent a substituted or unsubstituted alkyl group, a substituted or unsubstituted alkenyl group or a substituted or unsubstituted aryl group.

Each of the ring J and the groups represented by  $R^{32}$ ,  $R^{33}$  and  $R^{34}$  may further have a substituent. Examples of a substituent by which each of the ring J and the groups of  $R^{32}$ ,  $R^{33}$  and  $R^{34}$  may be substituted include the same substituents as each of the ring A and the substituents  $R^1$  to  $R^4$  in the formula (Y1) may have.

Examples of a preferred combination of the ring J and the substituents  $R^{32}$  to  $R^{34}$  in a dye represented by the formula (M3) include combinations wherein the ring J is a benzene ring substituted by an acylamino group having 2 to 8 carbon atoms,  $R^{32}$  is a substituted or unsubstituted alkyl group having 1 to 8 carbon atoms or an acyl group,  $R^{33}$  is a substituted or unsubstituted alkyl group having 1 to 8 carbon atoms or an allyl group, and  $R^{34}$  is a substituted or unsubstituted alkyl group having 1 to 8 carbon atoms or an allyl group.

In more preferred combinations of the ring J and the substituents  $R^{32}$  to  $R^{34}$ , the ring J is a benzene ring substituted by an acylamino group having 2 to 6 carbon atoms,  $R^{32}$  is a substituted or unsubstituted alkyl group having 1 to 6 carbon atoms or an acyl group,  $R^{33}$  is a substituted or unsubstituted alkyl group having 1 to 6 carbon atoms or an allyl group,  $R^{34}$  is a substituted or unsubstituted alkyl group having 1 to 6 carbon atoms or an allyl group, and  $R^{34}$  is a substituted or unsubstituted alkyl group having 1 to 6 carbon atoms or an allyl group.

In the most preferred combinations thereof, the ring J is a benzene ring substituted by an acylamino group having 2 to 4 carbon atoms,  $R^{32}$  is a substituted or unsubstituted alkyl group having 1 to 4 carbon atoms or an acyl group,  $R^{33}$  is a substituted or unsubstituted alkyl group having 1 to 4 carbon atoms or an allyl group, and  $R^{34}$  is a substituted or unsubstituted alkyl group having 1 to 4 carbon atoms or an allyl group.

Formula (M4)



In the formula (M4), the ring K represents a substituted or unsubstituted benzene ring, and  $R^{35}$ ,  $R^{36}$  and  $R^{37}$  each independently represent a substituted or unsubstituted alkyl group, a substituted or unsubstituted alkenyl group or a substituted or unsubstituted aryl group.

Each of the ring K and the groups represented by  $R^{35}$ ,  $R^{36}$  and  $R^{37}$  may further have a substituent. Examples of a substituent by which each of the ring K and the groups of  $R^{35}$ ,  $R^{36}$  and  $R^{37}$  may be substituted include the same substituents as each of the ring A and the substituents  $R^1$  to  $R^4$  in the formula (Y1) may have.

Examples of a preferred combination of the ring K and the substituents  $R^{35}$  to  $R^{37}$  in a dye represented by the formula (M4) include combinations wherein the ring K is a benzene ring substituted by an acylamino group having 2 to 8 carbon atoms,  $R^{35}$  is a substituted or unsubstituted alkyl group having 1 to 8 carbon atoms,  $R^{36}$  is a substituted or unsubstituted alkyl group having 1 to 8 carbon atoms or an allyl group, and  $R^{37}$  is a substituted or unsubstituted alkyl group having 1 to 8 carbon atoms or an allyl group.

In more preferred combinations of the ring K and the substituents  $R^{35}$  to  $R^{37}$ , the ring K is a benzene ring substituted by an acylamino group having 2 to 6 carbon atoms,  $R^{35}$  is a substituted or unsubstituted alkyl group having 1 to 6 carbon atoms,  $R^{36}$  is a substituted or unsubstituted alkyl group having 1 to 6 carbon atoms or an allyl group, and  $R^{37}$  is a substituted or unsubstituted alkyl group having 1 to 6 carbon atoms or an allyl group.

In the most preferred combinations thereof, the ring K is a benzene ring substituted by an acylamino group having 2 to 4 carbon atoms,  $R^{35}$  is a substituted or unsubstituted alkyl group having 1 to 4 carbon atoms,  $R^{36}$  is a substituted or unsubstituted alkyl group having 1 to 4 carbon atoms or an allyl group, and  $R^{37}$  is a substituted or unsubstituted alkyl group having 1 to 4 carbon atoms or an allyl group.

Formula (M5)



In the formula (M5),  $R^{38}$  and  $R^{39}$  each independently represent a substituted or unsubstituted alkyl group, a substituted or unsubstituted aryl group, or a substituted or unsubstituted heterocyclic group, and  $R^{40}$  and  $R^{41}$  each independently represent a substituted or unsubstituted alkyl group, a substituted or unsubstituted alkenyl group, or a substituted or unsubstituted aryl group.

Each of the groups represented by  $R^{38}$  to  $R^{41}$  may further have a substituent. Examples of a substituent by which  $R^{38}$  to  $R^{41}$  each may be substituted include the same substituents as each of the ring A and the substituents  $R^1$  to  $R^4$  in the formula (Y1) may have.

Examples of a preferred combination of the substituents  $R^{38}$  to  $R^{41}$  in a dye represented by the formula (M5) include combinations wherein  $R^{38}$  is a substituted or unsubstituted alkyl group having 1 to 8 carbon atoms or a substituted or unsubstituted aryl group having 6 to 10 carbon atoms,  $R^{39}$  is a substituted or unsubstituted alkyl group having 1 to 8 carbon atoms or a substituted or unsubstituted aryl group having 6 to 10 carbon atoms,  $R^{40}$  is a substituted or unsubstituted alkyl group having 1 to 8 carbon atoms or a substituted or unsub-

stituted aryl group having 6 to 10 carbon atoms, and R<sup>41</sup> is a substituted or unsubstituted alkyl group having 1 to 8 carbon atoms or a substituted or unsubstituted aryl group having 6 to 10 carbon atoms.

In more preferred combinations of the substituents R<sup>38</sup> to R<sup>41</sup>, R<sup>38</sup> is a substituted or unsubstituted alkyl group having 1 to 6 carbon atoms or a substituted or unsubstituted phenyl group, R<sup>39</sup> is a substituted or unsubstituted alkyl group having 1 to 6 carbon atoms or a substituted or unsubstituted phenyl group, R<sup>40</sup> is a substituted or unsubstituted alkyl group having 1 to 6 carbon atoms, and R<sup>41</sup> is a substituted or unsubstituted alkyl group having 1 to 6 carbon atoms.

In the most preferred combinations thereof, R<sup>38</sup> is a substituted or unsubstituted alkyl group having 1 to 4 carbon atoms or a substituted or unsubstituted phenyl group, R<sup>39</sup> is a substituted or unsubstituted alkyl group having 1 to 4 carbon atoms or a substituted or unsubstituted phenyl group, R<sup>40</sup> is a substituted or unsubstituted alkyl group having 1 to 4 carbon atoms, and R<sup>41</sup> is a substituted or unsubstituted alkyl group having 1 to 4 carbon atoms.



In the formula (M6), R<sup>42</sup> is a substituted or unsubstituted aryloxy group, R<sup>43</sup> is a hydrogen atom, or a substituted or unsubstituted aryloxy group, and R<sup>44</sup> is a hydroxyl group, or a substituted or unsubstituted amino group.

Each of the groups represented by R<sup>42</sup> and R<sup>43</sup> may further have a substituent. Examples of a substituent by which each of the groups of R<sup>42</sup> and R<sup>43</sup> may be substituted include the same substituents as each of the ring A and the substituents R<sup>1</sup> to R<sup>4</sup> in the formula (Y1) may have.

Examples of a preferred combination of the groups R<sup>42</sup> to R<sup>44</sup> in the dye represented by the formula (M6) include combinations wherein R<sup>42</sup> is a substituted or unsubstituted aryloxy group having 6 to 10 carbon atoms, R<sup>43</sup> is a hydrogen atom, or a substituted or unsubstituted aryloxy group having 6 to 10 carbon atoms, and R<sup>44</sup> is a hydroxyl group, or an unsubstituted amino group.

In more preferred combinations thereof, R<sup>42</sup> is a substituted or unsubstituted phenoxy group, R<sup>43</sup> is a hydrogen atom or a substituted or unsubstituted phenoxy group, and R<sup>44</sup> is a hydroxyl group, or an unsubstituted amino group.

In the most preferred combinations thereof, R<sup>42</sup> is a phenoxy group substituted by a substituted or unsubstituted amino group, or an unsubstituted phenoxy group, R<sup>43</sup> is a hydrogen atom, or a substituted or unsubstituted phenoxy group, and R<sup>44</sup> is a hydroxyl group, or an unsubstituted amino group.



In the formula (M7), the ring L represents a substituted or unsubstituted benzene ring; and R<sup>45</sup> and R<sup>46</sup> each independently represent a hydrogen atom, a substituted or unsubstituted alkyl group, a substituted or unsubstituted alkenyl group or a substituted or unsubstituted aryl group.

Each of the ring L and the groups represented by R<sup>45</sup> and R<sup>46</sup> may further have a substituent. Examples of a substituent by which each of the ring L and the groups of R<sup>45</sup> and R<sup>46</sup> may be substituted include the same substituents as each of the ring A and the substituents R<sup>1</sup> to R<sup>4</sup> in the formula (Y1) may have.

Examples of a preferred combination of the ring L and the substituents R<sup>45</sup> and R<sup>46</sup> include combinations wherein the ring L is a substituted or unsubstituted benzene ring, R<sup>45</sup> is a substituted or unsubstituted alkyl group having 1 to 8 carbon atoms, an allyl group, or a substituted or unsubstituted aryl group having 6 to 10 carbon atoms, and R<sup>46</sup> is a substituted or unsubstituted alkyl group having 1 to 8 carbon atoms, an allyl group, or a substituted or unsubstituted aryl group having 6 to 10 carbon atoms.

In more preferred combinations of the ring L and the substituents R<sup>45</sup> and R<sup>46</sup>, the ring L is a substituted or unsubstituted benzene ring, R<sup>45</sup> is a substituted or unsubstituted alkyl group having 1 to 6 carbon atoms, an allyl group, or a substituted or unsubstituted phenyl group, and R<sup>46</sup> is a substituted or unsubstituted alkyl group having 1 to 6 carbon atoms, an allyl group, or a substituted or unsubstituted phenyl group.

In the most preferred combinations thereof, the ring L is a benzene ring substituted by a methyl group, R<sup>45</sup> is an unsubstituted alkyl group having 1 to 4 carbon atoms, and R<sup>46</sup> is an alkyl group having 1 to 4 carbon atoms and a substituent(s).

Formula (M8)



In the formula (M8), the ring Q represents a substituted or unsubstituted benzene ring, R<sup>100</sup> represents a substituted or unsubstituted alkyl group, a substituted or unsubstituted aryl group, a substituted or unsubstituted alkoxy group, or a substituted or unsubstituted amino group, R<sup>101</sup> represents a substituted or unsubstituted alkyl group, or a substituted or unsubstituted aryl group, R<sup>102</sup> and R<sup>103</sup> each independently represent a hydrogen atom, a substituted or unsubstituted alkyl group, a substituted or unsubstituted alkenyl group, or a substituted or unsubstituted aryl group.

Each of the ring Q and the groups represented by R<sup>100</sup>, R<sup>101</sup>, R<sup>102</sup> and R<sup>103</sup> may further have a substituent. Examples of a substituent by which each of the ring Q and the groups of R<sup>100</sup>, R<sup>101</sup>, R<sup>102</sup> and R<sup>103</sup> may be substituted include the same substituents as each of the ring A and the substituents R<sup>1</sup> to R<sup>4</sup> in the formula (Y1) may have.

Examples of a preferred combination of the ring Q and the groups R<sup>100</sup> to R<sup>103</sup> in the dye represented by the formula (M8) include combinations wherein the ring Q is a substituted or unsubstituted benzene ring, R<sup>102</sup> is a substituted or unsubstituted alkyl group having 1 to 8 carbon atoms, an allyl group, or a substituted or unsubstituted aryl group having 6 to 10 carbon atoms, R<sup>103</sup> is a substituted or unsubstituted alkyl group having 1 to 8 carbon atoms, an allyl group, or a substi-

tuted or unsubstituted aryl group having 6 to 10 carbon atoms, R<sup>100</sup> is a substituted or unsubstituted amino group, or a substituted or unsubstituted alkoxy group, and R<sup>101</sup> is a substituted or unsubstituted alkyl group having 1 to 8 carbon atoms, or a substituted or unsubstituted aryl group having 6 to 10 carbon atoms.

In more preferred combinations thereof, the ring Q is a substituted or unsubstituted benzene ring, R<sup>102</sup> is a substituted or unsubstituted alkyl group having 1 to 6 carbon atoms, an allyl group, or a substituted or unsubstituted phenyl group, R<sup>103</sup> is a substituted or unsubstituted alkyl group having 1 to 6 carbon atoms, an allyl group, or a substituted or unsubstituted phenyl group, R<sup>100</sup> is a substituted or unsubstituted amino group, or a substituted or unsubstituted alkoxy group, and R<sup>101</sup> is a substituted or unsubstituted alkyl group having 1 to 6 carbon atoms, or a substituted or unsubstituted phenyl group.

In the most preferred combinations thereof, the ring Q is a substituted or unsubstituted benzene ring, R<sup>102</sup> is a substituted or unsubstituted alkyl group having 1 to 4 carbon atoms, or an allyl group, R<sup>103</sup> is a substituted or unsubstituted alkyl group having 1 to 4 carbon atoms, or an allyl group, R<sup>100</sup> is a substituted or unsubstituted amino group, or a substituted or unsubstituted alkoxy group, and R<sup>101</sup> is a substituted or unsubstituted phenyl group.

Formula (C1)



In the formula (C1), the ring M represents a substituted or unsubstituted benzene ring, R<sup>47</sup> represents a hydrogen atom or a halogen atom, R<sup>48</sup> represents a substituted or unsubstituted alkyl group, R<sup>49</sup> represents a substituted or unsubstituted acylamino group or a substituted or unsubstituted alkoxy carbonyl amino group, and R<sup>50</sup> and R<sup>51</sup> each independently represent a substituted or unsubstituted alkyl group, a substituted or unsubstituted alkenyl group or a substituted or unsubstituted aryl group.

Each of the ring M and the groups represented by R<sup>48</sup>, R<sup>49</sup>, R<sup>50</sup> and R<sup>51</sup> may further have a substituent. Examples of a substituent by which each of the ring M and the groups of R<sup>48</sup>, R<sup>49</sup>, R<sup>50</sup> and R<sup>51</sup> may be substituted include the same substituents as each of the ring A and the substituents R<sup>1</sup> to R<sup>4</sup> in the formula (Y1) may have.

Examples of a preferred combination of the ring M and the substituents R<sup>47</sup> to R<sup>51</sup> include combinations wherein the ring M is a benzene ring substituted by an alkyl group having 1 to 4 carbon atoms, a benzene ring substituted by a chlorine atom or an unsubstituted benzene ring, R<sup>47</sup> is a hydrogen atom, a chlorine atom or a bromine atom, R<sup>48</sup> is a substituted or unsubstituted alkyl group having 1 to 8 carbon atoms, R<sup>49</sup> is a substituted or unsubstituted acylamino group having 2 to 10 carbon atoms or a substituted or unsubstituted alkoxy carbonyl amino group having 2 to 10 carbon atoms, R<sup>50</sup> is a substituted or unsubstituted alkyl group having 1 to 8 carbon atoms, and R<sup>51</sup> is a substituted or unsubstituted alkyl group having 1 to 8 carbon atoms.

In preferred combinations of the ring M and the substituents R<sup>47</sup> to R<sup>51</sup>, the ring M is a benzene ring substituted by an

alkyl group having 1 to 2 carbon atoms or an unsubstituted benzene ring, R<sup>47</sup> is a hydrogen atom or a chlorine atom, R<sup>48</sup> is a substituted or unsubstituted alkyl group having 1 to 6 carbon atoms, R<sup>49</sup> is a substituted or unsubstituted acylamino group having 2 to 8 carbon atoms or a substituted or unsubstituted alkoxy carbonyl amino group having 2 to 8 carbon atoms, R<sup>50</sup> is a substituted or unsubstituted alkyl group having 1 to 6 carbon atoms, and R<sup>51</sup> is a substituted or unsubstituted alkyl group having 1 to 6 carbon atoms.

In the most preferred combinations thereof, the ring M is a benzene ring substituted by a methyl group or an unsubstituted benzene ring, R<sup>47</sup> is a hydrogen atom or a chlorine atom, R<sup>48</sup> is a substituted or unsubstituted alkyl group having 1 to 6 carbon atoms, R<sup>49</sup> is a substituted or unsubstituted acylamino group having 2 to 6 carbon atoms or a substituted or unsubstituted alkoxy carbonyl amino group having 2 to 6 carbon atoms, R<sup>50</sup> is a substituted or unsubstituted alkyl group having 1 to 4 carbon atoms, and R<sup>51</sup> is a substituted or unsubstituted alkyl group having 1 to 4 carbon atoms.

Formula (C2)



In the formula (C2), the ring N represents a substituted or unsubstituted benzene ring, R<sup>52</sup> represents a hydrogen atom, a substituted or unsubstituted acylamino group, a substituted or unsubstituted alkoxy carbonyl group, or a substituted or unsubstituted carbamoyl group, and R<sup>53</sup> and R<sup>54</sup> each independently represent a substituted or unsubstituted alkyl group, a substituted or unsubstituted alkenyl group, or a substituted or unsubstituted aryl group.

Each of the ring N and the groups represented by R<sup>52</sup>, R<sup>53</sup> and R<sup>54</sup> may further have a substituent. Examples of a substituent by which each of the ring N and the groups of R<sup>52</sup>, R<sup>53</sup> and R<sup>54</sup> may be substituted include the same substituents as each of the ring A and the substituents R<sup>1</sup> to R<sup>4</sup> in the formula (Y1) may have.

Examples of a preferred combination of the ring N and the groups R<sup>52</sup> to R<sup>54</sup> in the dye represented by the formula (C2) include combinations wherein the ring N is a benzene ring substituted by an alkyl group having 1 to 8 carbon atoms, a benzene ring substituted by an alkoxy group having 1 to 8 carbon atoms, or an unsubstituted benzene ring, R<sup>52</sup> is a hydrogen atom, a substituted or unsubstituted acylamino group having 2 to 10 carbon atoms, a substituted or unsubstituted alkoxy carbonyl group having 2 to 10 carbon atoms, or a substituted or unsubstituted carbamoyl group having 1 to 10 carbon atoms, R<sup>53</sup> is a substituted or unsubstituted alkyl group having 1 to 8 carbon atoms, and R<sup>54</sup> is a substituted or unsubstituted alkyl group having 1 to 8 carbon atoms.

In more preferred combinations thereof, the ring N is a benzene ring substituted by an alkyl group having 1 to 6 carbon atoms, a benzene ring substituted by an alkoxy group having 1 to 6 carbon atoms, or an unsubstituted benzene ring, R<sup>52</sup> is a hydrogen atom, a substituted or unsubstituted acylamino group having 2 to 8 carbon atoms, a substituted or unsubstituted alkoxy carbonyl group having 2 to 8 carbon atoms, or a substituted or unsubstituted carbamoyl group

having 1 to 8 carbon atoms,  $R^{53}$  is a substituted or unsubstituted alkyl group having 1 to 6 carbon atoms, and  $R^{54}$  is a substituted or unsubstituted alkyl group having 1 to 6 carbon atoms.

In the most preferred combinations thereof, the ring N is a benzene ring substituted by an alkyl group having 1 to 4 carbon atoms, a benzene ring substituted by an alkoxy group having 1 to 4 carbon atoms, or an unsubstituted benzene ring,  $R^{52}$  is a hydrogen atom, a substituted or unsubstituted acylamino group having 2 to 6 carbon atoms, a substituted or unsubstituted alkoxy carbonyl group having 2 to 6 carbon atoms, or a substituted or unsubstituted carbamoyl group having 1 to 6 carbon atoms,  $R^{53}$  is a substituted or unsubstituted alkyl group having 1 to 4 carbon atoms, and  $R^{54}$  is a substituted or unsubstituted alkyl group having 1 to 4 carbon atoms.



Formula (C3)

In the formula (C3),  $R^{55}$  and  $R^{56}$  each independently represent an alkyl group, or a substituted or unsubstituted aryl group.

Each of the groups represented by  $R^{55}$  and  $R^{56}$  may further have a substituent. Examples of a substituent by which each of the groups of  $R^{55}$  and  $R^{56}$  may be substituted include the same substituents as each of the ring A and the substituents  $R^1$  to  $R^4$  in the formula (Y1) may have.

Examples of a preferred combination of the substituents  $R^{55}$  and  $R^{56}$  in a dye represented by the formula (C3) include combinations wherein  $R^{55}$  is a substituted or unsubstituted alkyl group having 1 to 8 carbon atoms or a substituted or unsubstituted aryl group having 6 to 10 carbon atoms,  $R^{56}$  is a substituted or unsubstituted alkyl group having 1 to 8 carbon atoms or a substituted or unsubstituted aryl group having 6 to 10 carbon atoms.

In more preferred combinations of the substituents  $R^{55}$  and  $R^{56}$ ,  $R^{55}$  is a substituted or unsubstituted alkyl group having 1 to 6 carbon atoms or a substituted or unsubstituted phenyl group,  $R^{56}$  is a substituted or unsubstituted alkyl group having 1 to 6 carbon atoms or a substituted or unsubstituted phenyl group.

In the most preferred combinations thereof,  $R^{55}$  is a substituted or unsubstituted alkyl group having 1 to 4 carbon atoms,  $R^{56}$  is a substituted or unsubstituted alkyl group having 1 to 4 carbon atoms or a substituted or unsubstituted phenyl group.

Formula (C4)



10

In the formula (C4), the ring O represents a substituted or unsubstituted benzene ring, and  $R^{57}$  and  $R^{58}$  each independently represent a substituted or unsubstituted alkyl group, a substituted or unsubstituted alkenyl group, or a substituted or unsubstituted aryl group.

Each of the ring O and the groups represented by  $R^{57}$  and  $R^{58}$  may further have a substituent. Examples of a substituent by which each of the ring O and the groups of  $R^{57}$  and  $R^{58}$  may be substituted include the same substituents as each of the ring A and the substituents  $R^1$  to  $R^4$  in the formula (Y1) may have.

Examples of a preferred combination of the ring O and the groups  $R^{57}$  and  $R^{58}$  in the dye represented by the formula (C4) include combinations wherein the ring O is a benzene ring substituted by an alkyl group having 1 to 8 carbon atoms, a benzene ring substituted by an alkoxy group having 1 to 8 carbon atoms, or an unsubstituted benzene ring,  $R^{57}$  is a substituted or unsubstituted alkyl group having 1 to 8 carbon atoms, and  $R^{58}$  is a substituted or unsubstituted alkyl group having 1 to 8 carbon atoms.

In more preferred combinations thereof, the ring O is a benzene ring substituted by an alkyl group having 1 to 6 carbon atoms, a benzene ring substituted by an alkoxy group having 1 to 6 carbon atoms, or an unsubstituted benzene ring,  $R^{57}$  is a substituted or unsubstituted alkyl group having 1 to 6 carbon atoms, and  $R^{58}$  is a substituted or unsubstituted alkyl group having 1 to 6 carbon atoms.

In the most preferred combinations thereof, the ring O is a benzene ring substituted by an alkyl group having 1 to 4 carbon atoms, a benzene ring substituted by an alkoxy group having 1 to 4 carbon atoms, or an unsubstituted benzene ring,  $R^{57}$  is a substituted or unsubstituted alkyl group having 1 to 4 carbon atoms, and  $R^{58}$  is a substituted or unsubstituted alkyl group having 1 to 4 carbon atoms.

Specific examples of compounds as the dyes represented by the formulae (Y1) to (Y9), (M1) to (M8) and (C1) to (C4), which can be preferably used in the invention, are illustrated below. However, the dyes represented by the formulae (Y1) to (Y9), (M1) to (M8) and (C1) to (C4) used in the invention should not be restrictedly interpreted by the specific examples illustrated below.

TABLE 1

| The dyes represented by the formula (Y1) |        |       |       |        |        |
|------------------------------------------|--------|-------|-------|--------|--------|
| Examples of compounds                    | Ring A | $R^1$ | $R^2$ | $R^3$  | $R^4$  |
| Y1-1                                     |        | Ethyl | Ethyl | Ethoxy | Phenyl |

TABLE 1-continued

| The dyes represented by the formula (Y1) |        |                |                |                |                |
|------------------------------------------|--------|----------------|----------------|----------------|----------------|
| Examples of compounds                    | Ring A | R <sup>1</sup> | R <sup>2</sup> | R <sup>3</sup> | R <sup>4</sup> |
| Y1-2                                     |        | Ethyl          | Ethyl          | Dimethylamino  | Phenyl         |
| Y1-3                                     |        | n-Propyl       | n-Propyl       | Ethoxy         | Phenyl         |
| Y1-4                                     |        | n-Butyl        | n-Butyl        | Ethoxy         | Phenyl         |

TABLE 2

| The dyes represented by the formula (Y2) |                |                |                |                |                |
|------------------------------------------|----------------|----------------|----------------|----------------|----------------|
| Examples of compounds                    | R <sup>5</sup> | R <sup>6</sup> | R <sup>7</sup> | R <sup>8</sup> | R <sup>9</sup> |
| Y2-1                                     | Ethyl          | Methyl         | Methyl         | Dimethylamino  | Phenyl         |
| Y2-2                                     | n-Propyl       | Methyl         | Methyl         | Dimethylamino  | Phenyl         |
| Y2-3                                     | Allyl          | Methyl         | Methyl         | Dimethylamino  | Phenyl         |
| Y2-4                                     | Ethyl          | Methyl         | Methyl         | Ethoxy         | Phenyl         |

TABLE 3

| The dyes represented by the formula (Y3) |                 |                 |                       |
|------------------------------------------|-----------------|-----------------|-----------------------|
| Examples of compounds                    | R <sup>10</sup> | R <sup>11</sup> | R <sup>12</sup>       |
| Y3-1                                     | Isopropyl       | Hydrogen        | Di-n-butyl-carbamoyl  |
| Y3-2                                     | Hydrogen        | Bromo           | Di-n-propyl-carbamoyl |

TABLE 4

| The dyes represented by the formula (Y4) |        |                 |                          |
|------------------------------------------|--------|-----------------|--------------------------|
| Examples of compounds                    | Ring B | R <sup>13</sup> | R <sup>14</sup>          |
| Y4-1                                     |        | t-Butyl         | Phenyl                   |
| Y4-2                                     |        | t-Butyl         | Methyl                   |
| Y4-3                                     |        | t-Butyl         | 4-(Ethoxycarbonyl)phenyl |

TABLE 5

| The dyes represented by the formula (Y5) |                 |                 |                 |                 |
|------------------------------------------|-----------------|-----------------|-----------------|-----------------|
| Examples of compounds                    | R <sup>15</sup> | R <sup>16</sup> | R <sup>17</sup> | R <sup>18</sup> |
| Y5-1                                     | Methyl          | Methyl          | Phenyl          | Phenyl          |
| Y5-2                                     | Methyl          | Methyl          | Methyl          | Methyl          |

TABLE 6

| The dyes represented by the formula (Y6) |        |        |        |
|------------------------------------------|--------|--------|--------|
| Examples of compounds                    | Ring C | Ring D | Ring E |
| Y6-1                                     |        |        |        |
| Y6-2                                     |        |        |        |

33

TABLE 7

| The dyes represented by the formula (Y7) |        |                 |                          |
|------------------------------------------|--------|-----------------|--------------------------|
| Examples of compounds                    | Ring F | R <sup>19</sup> | R <sup>20</sup>          |
| Y7-1                                     |        | n-Butyl         | Benzyl                   |
| Y7-2                                     |        | Ethyl           | 4-Cyclohexylphenoxyethyl |
| Y7-3                                     |        | Ethyl           | Phenethyl                |
| Y7-4                                     |        | n-Butyl         | $-C_2H_4-$               |

34

TABLE 8

| The dyes represented by the formula (Y8) |        |                 |                 |
|------------------------------------------|--------|-----------------|-----------------|
| Examples of compounds                    | Ring G | R <sup>21</sup> | R <sup>22</sup> |
| Y8-1                                     |        | Methyl          | s-Butyl         |
| Y8-2                                     |        | Methyl          | t-Pentyl        |

TABLE 9

| The dyes represented by the formula (Y9) |                 |
|------------------------------------------|-----------------|
| Examples of compounds                    | R <sup>23</sup> |
| Y9-1                                     | Ethyl           |
| Y9-2                                     | n-Propyl        |
| Y9-3                                     | n-Butyl         |

TABLE 10

| The dyes represented by the formula (M1) |        |                 |                 |                       |
|------------------------------------------|--------|-----------------|-----------------|-----------------------|
| Examples of compounds                    | Ring H | R <sup>24</sup> | R <sup>25</sup> | R <sup>26</sup>       |
| M1-1                                     |        | 2-Chlorophenyl  | Isopropyl       | n-Butyl               |
| M1-2                                     |        | 2-Chlorophenyl  | Isopropyl       | Acetoxyethyl          |
| M1-3                                     |        | 2-Chlorophenyl  | Isopropyl       | n-Butyl               |
|                                          |        |                 |                 | 4-Methoxyphenoxyethyl |

TABLE 11

| The dyes represented by the formula (M2) |        |                 |                 |                                 |
|------------------------------------------|--------|-----------------|-----------------|---------------------------------|
| Examples of compounds                    | Ring I | R <sup>28</sup> | R <sup>29</sup> | R <sup>30</sup> R <sup>31</sup> |
| M2-1                                     |        | t-Butyl         | 3-Methylphenyl  | Ethyl Ethyl                     |
| M2-2                                     |        | 2-Chlorophenyl  | Isopropyl       | n-Butyl Cyanoethyl              |

35

TABLE 12

| The dyes represented by the formula (M3) |        |                 |                 |                 |
|------------------------------------------|--------|-----------------|-----------------|-----------------|
| Examples of compounds                    | Ring J | R <sup>32</sup> | R <sup>33</sup> | R <sup>34</sup> |
| M3-1                                     |        | n-Butyl         | n-Butyl         | n-Butyl         |
| M3-2                                     |        | Allyl           | n-Propyl        | n-Propyl        |

TABLE 13

| The dyes represented by the formula (M4) |        |                 |                 |                 |
|------------------------------------------|--------|-----------------|-----------------|-----------------|
| Examples of compounds                    | Ring K | R <sup>35</sup> | R <sup>36</sup> | R <sup>37</sup> |
| M4-1                                     |        | Methyl          | Ethyl           | Benzyl          |
| M4-2                                     |        | Methyl          | Ethyl           | Benzyl          |

TABLE 14

| The dyes represented by the formula (M5) |                 |                 |                 |                 |
|------------------------------------------|-----------------|-----------------|-----------------|-----------------|
| Examples of compounds                    | R <sup>38</sup> | R <sup>39</sup> | R <sup>40</sup> | R <sup>41</sup> |
| M5-1                                     | Methyl          | t-Butyl         | Ethyl           | Ethyl           |
| M5-2                                     | Phenyl          | t-Butyl         | Ethyl           | Ethyl           |
| M5-3                                     | Methyl          | t-Butyl         | n-Propyl        | n-Propyl        |
| M5-4                                     | Methyl          | t-Butyl         | n-Butyl         | n-Butyl         |

36

TABLE 15

| The dyes represented by the formula (M6) |                         |                 |                 |
|------------------------------------------|-------------------------|-----------------|-----------------|
| Examples of compounds                    | R <sup>42</sup>         | R <sup>43</sup> | R <sup>44</sup> |
| M6-1                                     | Phenoxy                 | Hydrogen        | Hydroxyl        |
| M6-2                                     | Phenoxy                 | Phenoxy         | Amino           |
| M6-3                                     | m-(N-Methylamino)phenyl | Hydrogen        | Hydroxyl        |

TABLE 16

| The dyes represented by the formula (M7) |        |                 |                 |
|------------------------------------------|--------|-----------------|-----------------|
| Examples of compounds                    | Ring L | R <sup>45</sup> | R <sup>46</sup> |
| M7-1                                     |        | Ethyl           | Ethyl           |
| M7-2                                     |        | n-Propyl        | n-Propyl        |

TABLE 17

| The dyes represented by the formula (M8) |        |                  |                  |                  |                  |
|------------------------------------------|--------|------------------|------------------|------------------|------------------|
| Examples of compounds                    | Ring Q | R <sup>100</sup> | R <sup>101</sup> | R <sup>102</sup> | R <sup>103</sup> |
| M8-1                                     |        | Dimethylamino    | Phenyl           | Ethyl            | Ethyl            |
| M8-2                                     |        | Dimethylamino    | Phenyl           | Ethyl            | Ethyl            |
| M8-3                                     |        | Ethoxy           | Phenyl           | Ethyl            | Ethyl            |
| M8-4                                     |        | Ethoxy           | Phenyl           | Ethyl            | Ethyl            |

TABLE 18

| The dyes represented by the formula (C1) |        |                 |                 |                          |                 |                 |
|------------------------------------------|--------|-----------------|-----------------|--------------------------|-----------------|-----------------|
| Examples of compounds                    | Ring M | R <sup>47</sup> | R <sup>48</sup> | R <sup>49</sup>          | R <sup>50</sup> | R <sup>51</sup> |
| Cl-1                                     |        | Chloro          | Methyl          | Acetylamino              | Ethyl           | Ethyl           |
| Cl-2                                     |        | Hydrogen        | Methyl          | Acetylamino              | Ethyl           | Ethyl           |
| Cl-3                                     |        | Chloro          | Hydrogen        | 3-Pyridine carbonylamino | n-Propyl        | n-Propyl        |
| Cl-4                                     |        | Chloro          | Methyl          | Acetylamino              | n-Propyl        | n-Propyl        |
| Cl-5                                     |        | Chloro          | Ethyl           | 2-Furoylamino            | Ethyl           | Ethyl           |

TABLE 19

| The dyes represented by the formula (C2) |        |                    |                 |                 |
|------------------------------------------|--------|--------------------|-----------------|-----------------|
| Examples of compounds                    | Ring N | R <sup>52</sup>    | R <sup>53</sup> | R <sup>54</sup> |
| C2-1                                     |        | Dimethyl-carbamoyl | Ethyl           | Benzyl          |
| C2-2                                     |        | Acetylamino        | Ethyl           | Ethyl           |
| C2-3                                     |        | Hydrogen           | Ethyl           | Isopropyl       |
| C2-4                                     |        | Ethoxy-carbonyl    | Ethyl           | Ethyl           |
| C2-5                                     |        | Hydrogen           | Ethyl           | Ethyl           |

TABLE 20

| The dyes represented by the formula (C3) |                 |                 |
|------------------------------------------|-----------------|-----------------|
| Examples of compounds                    | R <sup>55</sup> | R <sup>56</sup> |
| C3-1                                     | Isopropyl       | Isopropyl       |
| C3-2                                     | Methyl          | m-Tolyl         |
| C3-3                                     | m-Tolyl         | m-Tolyl         |

TABLE 21

| The dyes represented by the formula (C4) |                 |                 |
|------------------------------------------|-----------------|-----------------|
| Examples of compounds                    | R <sup>57</sup> | R <sup>58</sup> |
| C4-1                                     | Ethyl           | Ethyl           |
| C4-2                                     | n-Propyl        | n-Propyl        |
| C4-3                                     | n-Butyl         | n-Butyl         |

## (Binder)

55 The resin binder contained in the dye layer in the invention may be known one. Examples thereof include acrylic resins such as polyacrylonitrile, polyacrylate, and polyacrylamide; polyvinyl acetal resins such as polyvinyl acetoacetal, and polyvinyl butyral; cellulose resins such as ethylcellulose, hydroxyethylcellulose, ethylhydroxycellulose, hydroxypropylcellulose, ethylhydroxyethylcellulose, methylcellulose, cellulose acetate, cellulose acetate butyrate, cellulose acetate propionate, cellulose nitrate, other modified cellulose resins, nitrocellulose, and ethylhydroxyethylcellulose; other resins such as polyurethane resin, polyamide resin, polyester resin, polycarbonate resin, phenoxy resin, phenol resin, and epoxy resin; and various elastomers. The dye layer may be made of at least one resin selected from the above-mentioned group.

These may be used alone, or two or more thereof may be used in the form of a mixture or copolymer. These may be crosslinked with various crosslinking agents.

The binder in the invention is preferably a cellulose resin or a polyvinyl acetal resin, more preferably a polyvinyl acetal resin. In the invention, the binder resin is in particular preferably polyvinyl acetoacetal resin, or polyvinyl butyral resin.

In the heat-sensitive transfer sheet of the invention, a dye barrier layer may be formed between the dye layer and the base film.

The surface of the base film may be subjected to treatment for easy adhesion to improve the wettability and the adhesive property of the coating liquid. Examples of the treatment include corona discharge treatment, flame treatment, ozone treatment, ultraviolet treatment, radial ray treatment, surface-roughening treatment, chemical agent treatment, vacuum plasma treatment, atmospheric plasma treatment, primer treatment, grafting treatment, and other known surface modifying treatments.

An easily-adhesive layer may be formed on the base film by coating. Examples of the resin used in the easily-adhesive layer include polyester resins, polyacrylate resins, polyvinyl acetate resins, vinyl resins such as polyvinyl chloride resin and polyvinyl alcohol resin, polyvinyl acetal resins such as polyvinyl acetoacetal and polyvinyl butyral, polyether resins, polyurethane resins, styrene acrylate resins, polyacrylamide resins, polyamide resins, polystyrene resins, polyethylene resins, and polypropylene resins.

When a film used for the base film is formed by melt extrusion, it is allowable to subject a non-drawn film to coating treatment followed by drawing treatment.

The above-mentioned treatments may be used in combination of two or more thereof.

(Transferable Protective Layer Laminate)

In the invention, a transferable protective layer laminate is preferably formed in area order onto the heat-sensitive transfer sheet. The transferable protective layer laminate is used to protect a heat-transferred image with a protective layer composed of a transparent resin, thereby to improve durability such as scratch resistance, light-fastness, and resistance to weather. This laminate is effective for a case where the transferred dye is insufficient in image durabilities such as light resistance, scratch resistance, and chemical resistance in the state that the dye is naked in the surface of an image-receiving sheet.

The transferable protective layer laminate can be formed by forming, onto a support, a releasing layer, a protective layer and an adhesive layer in this order (i.e., in the layer-described order) successively. The protective layer may be formed by plural layers. In the case where the protective layer also has functions of other layers, the releasing layer and the adhesive layer can be omitted. It is also possible to use a base film on which an easy adhesive layer has already been formed.

(Transferable Protective Layer)

As a transferable protective layer-forming resin, preferred are resins that are excellent in scratch resistance, chemical resistance, transparency and hardness. Examples of the resin include polyester resins, polystyrene resins, acrylic resins, polyurethane resins, acrylic urethane resins, silicone-modified resins of the above-described resins, ultraviolet-shielding resins, mixtures of these resins, ionizing radiation-curable resins, and ultraviolet-curing resins. Particularly preferred are polyester resins and acrylic resins.

These resins may be crosslinked with various crosslinking agents.

(Transferable Protective Layer Resin)

As the acrylic resin, use can be made of polymers derived from at least one monomer selected from conventionally known acrylate monomers and methacrylate monomers.

5 Other monomers than these acrylate-series monomers, such as styrene and acrylonitrile may be co-polymerized with said acryl-series monomers. A preferred monomer is methyl methacrylate. It is preferred that methyl methacrylate is contained in terms of preparation mass ratio of 50 mass % or more in the polymer.

The acrylic resin in the invention preferably has a molecular weight of 20,000 or more and 100,000 or less.

15 The polyester resin in the invention may be a saturated polyester resin known in the prior art. As the above-described polyester resin, a preferable glass transition temperature ranges from 50° C. to 120° C., and a preferable molecular weight ranges from 2,000 to 40,000. A molecular weight ranging from 4,000 to 20,000 is more preferred, because 20 so-called "foil-off" properties at the time of transfer of the protective layer are improved.

(Ultraviolet Absorbent)

25 In the protective layer transferring sheet in the invention, an ultraviolet absorbent may be incorporated into the protective layer and/or the adhesive layer. The ultraviolet absorbent may be an inorganic ultraviolet absorbent or organic ultraviolet absorbent known in the prior art.

30 As the organic ultraviolet absorbing agents, use as the ultraviolet-shielding resin can be made of non-reactive ultraviolet absorbing agents such as salicylate-series, benzophenone-series, benzotriazole-series, triazine-series, substituted acrylonitrile-series, and hindered amine-series ultraviolet absorbing agents; and copolymers or graft polymers of thermoplastic resins (e.g., acrylic resins) and activated products 35 obtained by introducing to the above-described non-reactive ultraviolet absorbing agents; addition-polymerizable double bonds originated from a vinyl group, an acryroyl group, a methacryroyl group, or the like, or alternatively by introducing thereto other types of groups such as an alcoholic 40 hydroxyl group, an amino group, a carboxyl group, an epoxy group, and an isocyanate group. In addition, disclosed is a method of obtaining ultraviolet-shielding resins by the steps of dissolving ultraviolet absorbing agents in a monomer or oligomer of the resin to be used in the protective layer, and 45 then polymerizing the monomer or oligomer (JP-A-2006-21333). In this case, the ultraviolet absorbing agents may be non-reactive.

50 Of these ultraviolet absorbing agents, preferred are benzophenone-series, benzotriazole-series, and triazine-series ultraviolet absorbing agents. It is preferred that these ultraviolet absorbers are used in combination so as to cover an effective ultraviolet absorption wavelength region according to characteristic properties of the dye that is used for image formation. Besides, in the case of non-reactive ultraviolet 55 absorbers, it is preferred to use a mixture of two or more kinds of ultraviolet absorbers each having a different structure from each other so as to prevent the ultraviolet absorbers from precipitation.

Examples of commercially available ultraviolet absorbing agents include TINUVIN-P (trade name, manufactured by Ciba-Geigy), JF-77 (trade name, manufactured by JOHOKU CHEMICAL CO., LTD.), SEESORB 701 (trade name, manufactured by SHIRAI SHI CALCIUM KAISHA, LTD.), SUMISOUB 200 (trade name, manufactured by Sumitomo 60 Chemical Co., Ltd.), BIOSOUP 520 (trade name, manufactured by KYODO CHEMICAL CO., LTD.), and ADKSTAB LA-32 (trade name, manufactured by ADEKA).

41

## (Formation of the Transferable Protective Layer)

The method for forming the protective layer, which depends on the kind of the resin to be used, may be the same method for forming the dye layer. The protective layer preferably has a thickness of 0.5 to 10  $\mu\text{m}$ .

## (Releasing Layer)

In a case where the protective layer is not easily peeled from the support in the protective layer transferring sheet when the image is thermally transferred, a releasing layer may be formed between the support and the protective layer. A peeling layer may be formed between the transferable protective layer and the releasing layer. The releasing layer may be formed by painting a coating liquid by a method known in the prior art, such as gravure coating or gravure reverse coating, and then drying the painted liquid. The coating liquid contains at least one selected from, for example, waxes, silicone waxes, silicone resins, fluorine-contained resins, acrylic resins, polyvinyl alcohol resins, cellulose derivative resins, urethane resins, vinyl acetate resins, acryl vinyl ether resins, maleic anhydride resins, and copolymers of these resins. Of these resins, preferred are: acrylic resins, such as resin obtained by homopolymerizing a (meth)acrylic monomer such as acrylic acid or methacrylic acid, or obtained by copolymerizing a methacrylic monomer with a different monomer; or cellulose derivative resins. They are each excellent in adhesive property to the support, and releasing ability from the protective layer.

These resins may be crosslinked with various crosslinking agents. Moreover, ionizing radiation curable resin and ultraviolet curable resin may be used.

The releasing layer may be appropriately selected from a releasing layer which is transferred to a transferred-image-receiving member when the image is thermally transferred, a releasing layer which remains on the support side at that time, a releasing layer which is broken out by aggregation at that time, and other releasing layers. A preferred embodiment of the invention is an embodiment wherein the releasing layer remains on the support side at the time of the thermal transfer and the interface between the releasing layer and the thermally transferable protective layer becomes a protective layer surface after the thermal transfer since the embodiment is excellent in surface gloss, the transfer stability of the protective layer, and others. The method for forming the releasing layer may be a painting method known in the prior art. The releasing layer preferably has a thickness of about 0.5 to 5  $\mu\text{m}$  in the state that the layer is dried.

## (Adhesive Layer)

An adhesive layer may be formed, as the topmost layer of the transferable protective layer laminate, on the topmost surface of the protective layer. This makes it possible to make the adhesive property of the protective layer to a transferred-image-receiving member good.

## 2) Heat-Sensitive Transfer Image-Receiving Sheet

A heat-sensitive transfer image-receiving sheet (hereinafter also referred to merely as an image-receiving sheet) will be described in detail hereinafter. The image-receiving sheet, which is used to form an image by applying heat to this sheet and the heat-sensitive transfer sheet of the invention which are put on each other by means of a thermal printer head or the like, has a sheet having a support and at least one dye-receiving layer (hereinafter also referred to merely as a receiving layer) over the support. Between the support and the receiving layer may be formed an intermediate layer such as a heat insulating layer (porous layer), a gloss control layer, a white background adjusting layer, a charge control layer, an adhesive layer, or a primer layer. The image-receiving sheet pref-

42

erably has at least one heat insulating layer between the support and the receiving layer.

The dye-receiving layer and the intermediate layer are preferably formed by simultaneous multilayer-coating. If necessary, plural intermediate layers may be formed.

A curling control layer, a writing layer, or a charge-control layer may be formed on the backside of the support. Each of these layers may be applied using a usual method such as a roll coating, a bar coating, a gravure coating, and a gravure reverse coating.

## (Receiving Layer)

The image-receiving sheet has at least one receiving layer containing a thermoplastic polymer which can receive the dye. The receiving layer may contain an ultraviolet absorbent, a releasing agent, a lubricant, an antioxidant, a preservative, a surfactant, and other additives.

## (Thermoplastic Resin)

In the invention, a known thermoplastic resistance may be used for the receiving layer.

Preferred examples of the thermoplastic resin include polycarbonate, polyester, polyurethane, polyvinyl chloride and copolymers thereof, styrene-acrylonitrile copolymer, polycaprolactone, and mixtures thereof. Polyester, polyvinyl chloride and copolymers thereof, or mixtures thereof are more preferred. These polymers may be used alone or in a mixture form.

The above-exemplified polymers may be dissolved in a proper organic solvent such as methylethyl ketone, ethyl acetate, benzene, toluene, and xylene so that they can be coated on a support. Alternatively, they may be added to a water-based coating liquid as polymer latex so that they can be coated on a support. Polyester and polyvinyl chloride will be described in more detail hereinafter.

## (Polyester Polymers)

The polyester polymers are obtained by polycondensation of a dicarboxylic acid component (including a derivative thereof) and a diol component (including a derivative thereof). The polyester polymers may contain an aromatic ring and/or an aliphatic ring. As to the alicyclic polyester, those described in JP-A-5-238167 are useful from the viewpoints of ability to incorporate a dye and image stability.

In the present invention, as the polyester polymers, it is preferable to use polyester polymers obtained by polycondensation using at least one of the above-described dicarboxylic acid component and at least one of the above-described diol component, so that the thus-obtained polyester polymers could have a molecular weight (weight-average molecular weight (Mw)) of generally about 11,000 or more, preferably about 15,000 or more, and more preferably about 17,000 or more. If polyester polymers of too low molecular weight are used, elastic coefficient of the formed receptor layer becomes low and also it raises lack of thermal resistance. Resultantly, it sometimes becomes difficult to assure the releasing property of the heat-sensitive transfer sheet and the image-receiving sheet. A higher molecular weight is more preferable from a viewpoint of increase in elastic coefficient. The molecular weight is not limited in particular, so long as such failure does not occur that a higher molecular weight makes the polymer difficult to be dissolved in a solvent for a coating solution at the time of forming the receptor layer, or that an adverse effect arises in adhesive properties of the receptor layer to the support after coating and drying the receptor layer. However, the molecular weight is preferably about 25,000 or less, and at highest a degree of about 30,000. The polyester polymers may be synthesized according to a known method.

As the polyester which is of a saturated type, for example, the following may be used: VYLONAL MD-1200, VYLONAL MD-1220, VYLONAL MD-1245, VYLONAL MD-1250, VYLONAL MD-1500, VYLONAL MD-1930, or VYLONAL MD-1985, which is a trade name, manufactured by Toyobo Co., Ltd.

(Vinyl Chloride-Series Polymers)

The vinyl chloride-series polymers, particularly a copolymer using vinyl chloride, used in the receptor layer are explained in more detail.

The monomer which is copolymerized with vinyl chloride is not particularly limited as far as the monomer is copolymerizable with vinyl chloride. Particularly preferred is vinyl acetate, an acrylic acid ester or a methacrylic acid ester. Very good examples of the copolymer include vinyl chloride-vinyl acetate copolymer, vinyl chloride-acrylic acid ester copolymer, and vinyl chloride-methacrylic acid ester copolymer. The copolymers are each not necessarily a copolymer composed only of vinyl chloride and the above-mentioned preferred monomer (i.e., vinyl acetate, an acrylic acid ester or a methacrylic acid ester), and each contain a component other than these monomers, such as a vinyl alcohol component or maleic component, as far as the attainment of the objects of the invention is not hindered. Examples of the other component, which may constitute a copolymer composed mainly of vinyl chloride and the preferred monomer(s), include vinyl alcohol, vinyl alcohol derivatives such as vinyl propionate, acrylic acid, methacrylic acid, (meth)acrylic acid derivatives such as methyl, ethyl, propyl, butyl and 2-ethylhexyl esters of the acids, maleic acid, maleic acid derivatives such as diethyl maleate, dibutyl maleate and diethyl maleate, vinyl ether derivatives such as methyl vinyl ether, butyl vinyl ether and 2-ethylhexyl vinyl ether, acrylonitrile, methacrylonitrile, and styrene. The component ratio between vinyl chloride and the preferred monomer(s) in the copolymer may be an arbitrary ratio. The ratio by mass of the vinyl chloride component in the copolymer is preferably 50 mass % or more. The ratio by mass of the component other than vinyl chloride and the preferred monomers is preferably 10 mass % or less.

Examples of the vinyl chloride-vinyl acetate copolymer include VINYBRANE 240, VINYBRANE 601, VINYBRANE 602, VINYBRANE 380, VINYBRANE 386, VINYBRANE 410, and VINYBRANE 550, each of which is a trade name, manufactured by Nissin Chemical Industry Co., Ltd.

Examples of the vinyl chloride-acrylic acid ester copolymer include VINYBRANE 270, VINYBRANE 276, VINYBRANE 277, VINYBRANE 609, VINYBRANE 680, VINYBRANE 690, and VINYBRANE 900, each of which is a trade name, manufactured by Nissin Chemical Industry Co., Ltd. (Latex Polymer)

In the present invention, latex polymers can also be preferably used. Hereinafter, the latex polymer will be explained.

In the heat-sensitive transfer image-receiving sheet that can be used in the present invention, the latex polymer used in the receptor layer is a dispersion in which hydrophobic polymers are dispersed as fine particles in a water-soluble dispersion medium. The dispersed particles preferably have a mean particle size (diameter) of about 1 to 50,000 nm, more preferably about 5 to 1,000 nm.

The latex polymer that can be used in the present invention may be latex of the so-called core/shell type, other than ordinary latex polymer of a uniform structure. When using a core/shell type latex polymer, it is preferred in some cases that the core and the shell have different glass transition temperatures. The glass transition temperature (Tg) of the latex polymer that can be used in the present invention is preferably

-30° C. to 130° C., more preferably 0° C. to 120° C., and further more preferably 10° C. to 100° C.

In the present invention, it is preferable to prepare the receptor layer by applying an aqueous type coating solution and then drying it. The "aqueous type" so-called here means that 60% by mass or more of the solvent (dispersion medium) of the coating solution is water. As a component other than water in the coating solution, a water miscible organic solvent may be used, such as methyl alcohol, ethyl alcohol, isopropyl alcohol, dimethylformamide, ethyl acetate, diacetone alcohol, furfuryl alcohol, benzyl alcohol, diethylene glycol monoethyl ether, and oxyethyl phenyl ether.

In combination with the above-described latex polymer that can be used in the present invention, any polymer can be used. The polymer that can be used in combination is preferably transparent or translucent, and colorless. The polymer may be a natural resin, polymer, or copolymer; a synthetic resin, polymer, or copolymer; or another film-forming medium; and specific examples include gelatins, polyvinyl alcohols, hydroxyethylcelluloses, cellulose acetates, cellulose acetate butyrates, polyvinylpyrrolidones.

The glass transition temperature (Tg) of the binder that can be used in the present invention is preferably in the range of -30° C. to 90° C., more preferably -10° C. to 85° C., still more preferably 0° C. to 70° C., in view of film-forming properties (brittleness for working) and image preservability. A blend of two or more types of polymers can be used as the binder. When a blend of two or more polymers is used, the average Tg obtained by summing up the Tg of each polymer weighted by its proportion, is preferably within the foregoing range. Also, when phase separation occurs or when a core-shell structure is adopted, the weighted average Tg is preferably within the foregoing range.

[Releasing Agent]

In the present invention, a releasing agent may be used in the receptor layer in order to keep more securely the releasing property between the heat-sensitive transfer sheet and the image-receiving sheet at the time of printing images.

As the releasing agent, solid waxes such as polyethylene wax and amide wax; silicone oil, phosphate-series compounds, fluorine-based surfactants, silicone-based surfactants and others including releasing agents known in the technical fields concerned may be used. Among these, fluorine-series compounds typified by fluorine-based surfactants, silicone-based surfactants and silicone-series compounds such as silicone oil and/or its hardened products are preferably used.

In the present invention, the amount of the receptor layer to be applied is preferably 0.5 to 10 g/m<sup>2</sup> (solid basis, hereinafter, the amount to be applied in the present specification is a value on solid basis unless otherwise noted).

<Releasing Layer>

In the case where the hardened modified silicone oil is not added to the receptor layer, the silicone oil may be added to a releasing layer provided on the receptor layer. In this case, the receptor layer may be provided using at least one of the above-described thermoplastic resins. Besides, a receptor layer to which silicone is added may be used. The releasing layer contains a hardened modified silicone oil. A kind of the silicone to be used and a method of using the silicone are the same as for use in the receptor layer. Also, in the case where a catalyst or a retardant is used, the above described descriptions related to addition of these additives to the receptor layer may be applied. The releasing layer may be formed using only a silicone, or alternatively a mixture of a silicone and a binder

60 to 65

resin having a good compatibility therewith. A thickness of the releasing layer is generally in the range of about 0.001 to about 1 g/m<sup>2</sup>.

(Hollow Polymer)

In the image-receiving sheet used in the invention, its heat insulating layer preferably contains a hollow polymer and a water-soluble polymer.

The hollow polymer particles in the present invention are polymer particles having independent pores inside of the particles. Examples of the hollow polymer particles include (1) non-foaming type hollow particles obtained in the following manner: a dispersion medium, such as water, is contained inside of a capsule wall formed of a polystyrene, acryl resin, or styrene/acryl resin, and, after a coating solution is applied and dried, the dispersion medium in the particles is vaporized out of the particles, with the result that the inside of each particle forms a hollow; (2) foaming type microballoons obtained in the following manner: a low-boiling point liquid, such as butane and pentane, is encapsulated in a resin constituted of any one of polyvinylidene chloride, polyacrylonitrile, polyacrylic acid, and polyacrylate, or their mixture or polymer, and after the resin coating material is applied, it is heated to expand the low-boiling point liquid inside of the particles, whereby the inside of each particle is made to be hollow; and (3) microballoons obtained by foaming the above (2) under heating in advance, to make hollow polymer particles.

The particle size of the hollow polymer particles is preferably 0.1 to 20 µm, more preferably 0.1 to 5.0 µm, further preferably 0.2 to 3.0 µm, particularly preferably 0.3 to 1.0 µm.

The porosity of the hollow polymer is preferably from about 20 to 70%, more preferably from about 20 to 50%. The porosity of the hollow polymer is the ratio of the volume of the pores to that of the particles.

The glass transition temperature (Tg) of the hollow polymer particles is preferably 70° C. or higher, more preferably 90° C. or higher. These hollow polymer particles may be used in combinations of two or more of those, according to the need.

Such hollow polymer particles are commercially available. Specific examples of the above (1) include Rohpake 1055, manufactured by Rohm and Haas Co.; Boncoat PP-1000, manufactured by Dainippon Ink and Chemicals, Incorporated; SX866(B), manufactured by JSR Corporation; and Nippol MH5055, manufactured by Nippon Zeon (all of these product names are trade names). Specific examples of the above (2) include F-30, and F-50, manufactured by Matsuno Yushi-Seiyaku Co., Ltd. (all of these product names are trade names). Specific examples of the above (3) include F-30E, manufactured by Matsumoto Yushi-Seiyaku Co., Ltd, and Expance 461DE, 551DE, and 551DE20, manufactured by Nippon Ferrite (all of these product names are trade names). Among these, the hollow polymer particles of the above (1) may be preferably used.

(Water-Soluble Polymer)

The binder for the heat insulating layer may be a water-soluble polymer. The water-soluble polymer that can be used in the heat insulating layer is preferably a polymer used together with polymer latex. Herein, the "water-soluble polymer" means a polymer which dissolves, in 100 g water at 20° C., in an amount of preferably 0.05 g or more, more preferably 0.1 g or more, further preferably 0.5 g or more, and particularly preferably 1 g or more.

In the invention, the water-soluble polymer is preferably a polyvinyl alcohol, or gelatin, most preferably gelatin.

Further, the water-soluble polymers that are contained in the heat insulation layer may be cross-linked with a hardener

in order to regulate cushion properties and film strength. Preferable examples of the hardener that can be used in the present invention include H-1, 4, 6, 8, and 14 in JP-A-1-214845 in page 17; compounds (H-1 to H-54) represented by one of the formulae (VII) to (XII) in U.S. Pat. No. 4,618,573, columns 13 to 23; compounds (H-1 to H-76) represented by the formula (6) in JP-A-2-214852, page 8, the lower right (particularly, H-14); and compounds described in Claim 1 in U.S. Pat. No. 3,325,287.

10 <Support>

The support may be a coated paper sheet, a laminate paper sheet, or a synthetic paper sheet.

<Curl Control Layer, Writing Layer or Charge Control Layer>

15 In the heat-sensitive transfer image-receiving sheet used in the invention, a curl control layer, a writing layer or a charge control layer may be formed on the support surface (rear surface) reverse to the support surface on which the receiving layer is formed by painting.

20 3) Image-Forming

In the image-forming method (system) of the present invention, imaging is achieved by superposing a heat-sensitive transfer sheet on a heat-sensitive transfer image-receiving sheet so that a heat transfer layer of the heat-sensitive transfer sheet is in contact with a receptor layer of the heat-sensitive transfer image-receiving sheet and giving thermal energy in accordance with image signals given from a thermal head.

25 Specifically, image-forming can be achieved by the similar manner to that as described in, for example, JP-A-2005-88545. In the present invention, a printing time is preferably less than 15 seconds, and more preferably in the range of 3 to 12 seconds, and further preferably 3 to 7 seconds, from the viewpoint of shortening a time taken until a consumer gets a print.

30 In order to accomplish the above-described printing time, a line speed at the time of printing is preferably 1.0 msec/line or less, and further preferably 0.65 msec/line or less. Further, from the viewpoint of improvement in transfer efficiency as one of speeding-up conditions, the maximum ultimate temperature of the thermal head at the time of printing is preferably in the range of from 180° C. to 450° C., more preferably from 200° C. to 450° C., and furthermore preferably from 350° C. to 450° C.

35 45 The method of the present invention may be utilized for printers, copying machines and the like, which employs a heat-sensitive transfer recording system. As a means for providing heat energy in the thermal transfer, any of the conventionally known providing means may be used. For example, application of a heat energy of about 5 to 100 mJ/mm<sup>2</sup> by controlling recording time in a recording device such as a thermal printer (e.g. trade name: Video Printer VY-100, manufactured by Hitachi, Ltd.), sufficiently attains the expected result. Also, the heat-sensitive transfer image-receiving sheet for use in the present invention may be used in various applications enabling thermal transfer recording, such as heat-sensitive transfer image-receiving sheets in a form of thin sheets (cut sheets) or rolls; cards; and transmittable type manuscript-making sheets, by optionally selecting the type of support.

40 50 55 According to the invention, it is possible to provide a heat-sensitive transfer sheet which is restrained from being deformed in high-speed printing, thereby overcoming defects of printed images, and can simultaneously decrease the amount of materials adhering onto a thermal printer head, thereby restraining the sheet itself from being cut so as not to cause any abnormal step of the printer.

The present invention will be described in more detail based on the following examples, but the invention is not intended to be limited thereto. In the following Examples, the terms "part" and "%" are values by mass, unless they are indicated differently in particular.

## EXAMPLES

## (Production of Heat-Sensitive Transfer Sheets)

As a support, prepared was a polyester film, 4.5  $\mu\text{m}$  in thickness, having a single surface subjected to treatment for easy adhesion, and then a heat-resistant-lubricating-layer-coating liquid, which will be detailed later, was painted onto the surface of the film not subjected to the treatment for easy adhesion so that the solid coating amount would be 0.8 g/ $\text{m}^2$  after the liquid was dried. In the heat-resistant-lubricating-layer-coating liquid, the ratio by mole of reactive groups of polyisocyanate to those of the resin ( $-\text{NCO}/\text{OH}$ ) was 1.1. Immediately after the painting, the workpiece was dried at

100°C. in an oven for 1 minute, and subsequently subjected to heat treatment so as to conduct crosslinking reaction between the isocyanate and the polyol. In this way, the workpiece was cured.

5 Coating liquids, which will be detailed later, were used to form, onto the easily-adhesive layer painted surface of the thus-formed polyester film, individual heat-sensitive transfer layers in yellow, magenta and cyan, and a transferable protective layer laminate in area order by painting. In this way, a 10 heat-sensitive transfer sheet was produced. The solid coating amount in each of the heat-sensitive transfer layers (dye layers) was set to 0.9 g/ $\text{m}^2$ . Immediately after these were painted, the workpiece was dried at 100°C. in an oven for 1 minute.

In the formation of the transferable protective layer laminate, a releasing-layer-coating liquid was applied, and a protective-layer-coating liquid was applied thereon. The resultant was dried, and then an adhesive-layer-coating liquid was applied thereon. The resultant was then dried. In this way, a 15 heat-sensitive transfer sheet (101) was formed.

| Heat-resistant-lubricating-layer-coating liquid                                   |                 |
|-----------------------------------------------------------------------------------|-----------------|
| Acrylic polyol resin                                                              | 26.0 mass parts |
| Phosphate ester                                                                   | 9.8 mass parts  |
| (trade name: PLYSURF A208N, manufactured by Dai-ichi Kogyo Seiyaku Co., Ltd.)     |                 |
| Zinc stearylphosphate                                                             | 0.6 mass part   |
| Zinc stearate                                                                     | 0.6 mass part   |
| Polyisocyanate (50% solution)                                                     | 17.5 mass parts |
| (trade name: BIRNOCK D-750, manufactured by Dainippon Ink & Chemicals, Inc.)      |                 |
| Methyl ethyl ketone/toluene mixed solvent                                         | 70 mass parts   |
| Yellow-dye-coating liquid                                                         |                 |
| Dye compound (Y4-2)                                                               | 3.8 mass parts  |
| Dye compound (Y7-4)                                                               | 4.8 mass parts  |
| Polyvinylacetal resin                                                             | 7.6 mass parts  |
| (trade name: ESLEC KS-1, manufactured by Sekisui Chemical Co., Ltd.)              |                 |
| Polyvinylbutyral resin                                                            | 0.6 mass part   |
| (trade name: DENKA BUTYRAL #6000-C, manufactured by DENKI KAGAKU KOGYOU K. K.)    |                 |
| Releasing agent                                                                   | 0.05 mass part  |
| (trade name: X-22-3000T, manufactured by Shin-Etsu Chemical Co., Ltd.)            |                 |
| Releasing agent                                                                   | 0.03 mass part  |
| (trade name: TSF4701, manufactured by MOMENTIVE Performance Materials Japan LLC.) |                 |
| Matting agent                                                                     | 0.15 mass part  |
| (trade name: Flo-thene UF, manufactured by Sumitomo Seika Chemicals Co., Ltd.)    |                 |
| Methyl ethyl ketone/toluene mixed solvent                                         | 84 mass parts   |
| Magenta-dye-coating liquid                                                        |                 |
| Dye compound (M3-1)                                                               | 1.0 mass part   |
| Dye compound (M3-2)                                                               | 6.5 mass parts  |
| Dye compound (C1-2)                                                               | 0.3 mass part   |
| Polyvinylacetal resin                                                             | 7.5 mass parts  |
| (trade name: ESLEC KS-1, manufactured by Sekisui Chemical Co., Ltd.)              |                 |
| Polyvinylbutyral resin                                                            | 0.7 mass part   |
| (trade name: DENKA BUTYRAL #6000-C, manufactured by DENKI KAGAKU KOGYOU K. K.)    |                 |
| Releasing agent                                                                   | 0.05 mass part  |
| (trade name: X-22-3000T, manufactured by Shin-Etsu Chemical Co., Ltd.)            |                 |
| Releasing agent                                                                   | 0.03 mass part  |
| (trade name: TSF4701, manufactured by MOMENTIVE Performance Materials Japan LLC.) |                 |
| Matting agent                                                                     | 0.15 mass part  |
| (trade name: Flo-thene UF, manufactured by Sumitomo Seika Chemicals Co., Ltd.)    |                 |
| Methyl ethyl ketone/toluene mixed solvent                                         | 84 mass parts   |
| Cyan-dye-coating liquid                                                           |                 |
| Dye compound (C1-2)                                                               | 1.5 mass parts  |
| Dye compound (C3-1)                                                               | 7.7 mass parts  |
| Polyvinylacetal resin                                                             | 7.0 mass parts  |

-continued

(trade name: ESLEC KS-1, manufactured by Sekisui Chemical Co., Ltd.)

Polyvinylbutyral resin 1.2 mass part

(trade name: DENKA BUTYRAL #6000-C, manufactured by DENKI

KAGAKU KOGYOU K. K.)

Releasing agent 0.02 mass part

(trade name: X-22-3000T, manufactured by Shin-Etsu Chemical Co., Ltd.)

Releasing agent 0.02 mass part

(trade name: TSF4701, manufactured by MOMENTIVE Performance

Materials Japan LLC.)

Matting agent 0.1 mass part

(trade name: Flo-thene UF, manufactured by Sumitomo Seika Chemicals Co.,

Ltd.)

Methyl ethyl ketone/toluene mixed solvent 84 mass parts

(Transfer Protective Layer Laminate)

20

-continued

On the polyester film coated with the dye layers as described above, coating solutions of a releasing layer, a protective layer and an adhesive layer each having the following composition was coated, to form a transfer protective layer laminate. Coating amounts of the releasing layer, the protective layer and the adhesive layer after drying were 0.2 g/m<sup>2</sup>, 0.4 g/m<sup>2</sup> and 2.0 g/m<sup>2</sup>, respectively.

(UV-2)



Releasing-layer-coating liquid

30

Modified cellulose resin 5.0 mass parts  
(trade name: L-30, manufactured by  
DAICEL CHEMICAL INDUSTRIES, LTD.)  
Methyl ethyl ketone/toluene mixed solvent 95.0 mass parts  
Protective-layer-coating liquid

35 (UV-3)



Acrylic resin solution (Solid content: 40%) 90 mass parts  
(trade name: UNO-1, manufactured by  
Gifu Ceramics Limited)  
Methanol/isopropanol mixed solvent 10 mass parts  
Adhesive-layer-coating liquid

40

Acrylic resin 25 mass parts  
(trade name: DIANAL BR-77, manufactured by  
MITSUBISHI RAYON CO., LTD.)  
The following ultraviolet absorber UV-1 0.5 mass part  
The following ultraviolet absorber UV-2 2 mass parts  
The following ultraviolet absorber UV-3 0.5 mass part  
The following ultraviolet absorber UV-4 0.5 mass part  
PMMA fine particles 0.4 mass part  
(polymethyl methacrylate fine particles)  
Methyl ethyl ketone/toluene mixed solvent 70 mass parts

45 (UV-4)



60 Heat-sensitive transfer sheets (102) to (117) were each produced in the same way as in the production of the heat-sensitive transfer sheet (101) except that inorganic particles were incorporated into the heat-resistant lubricating layer.  
65 The structure of the inorganic particles in the heat-resistant lubricating layer of each of these heat-sensitive transfer sheets is shown in Table 22.

TABLE 22

| Inorganic particles in heat-resistant lubricating layer |                           |                    |                                                                    |                                     |                                |
|---------------------------------------------------------|---------------------------|--------------------|--------------------------------------------------------------------|-------------------------------------|--------------------------------|
| Sample name                                             | Material (Mohs' hardness) | Mean particle size | Mean ratio of particle maximum width to sphere equivalent diameter | Particulate form                    | Content by percentage (mass %) |
| 101                                                     | —                         | —                  | —                                                                  | —                                   | —                              |
| 102                                                     | Talc (1)                  | 3.8 $\mu\text{m}$  | 3.3                                                                | Tabular form                        | 0.6                            |
| 103                                                     | Magnesium oxide (4)       | 1.8 $\mu\text{m}$  | 1.4                                                                | Cubic form                          | 0.6                            |
| 104                                                     | Magnesium oxide (4)       | 1.1 $\mu\text{m}$  | 32.5                                                               | Needle form                         | 0.6                            |
| 105                                                     | Magnesium oxide (4)       | 1.2 $\mu\text{m}$  | 4.4                                                                | Tabular form                        | 0.6                            |
| 106                                                     | Magnesium oxide (4)       | 5.7 $\mu\text{m}$  | 12.8                                                               | Tabular form                        | 0.6                            |
| 107                                                     | Magnesium oxide (4)       | 3.5 $\mu\text{m}$  | 10.4                                                               | Tabular form                        | 0.6                            |
| 108                                                     | Magnesium oxide (4)       | 0.44 $\mu\text{m}$ | 5.5                                                                | Tabular form                        | 0.6                            |
| 109                                                     | Magnesium oxide (4)       | 0.23 $\mu\text{m}$ | 2.7                                                                | Tabular form                        | 0.6                            |
| 110                                                     | Magnesium carbonate (3.5) | 3.2 $\mu\text{m}$  | 12.8                                                               | Tabular form                        | 0.6                            |
| 111                                                     | Magnesium oxide (4)       | 1.3 $\mu\text{m}$  | 8.8                                                                | Mixture of needle and tabular forms | 0.6                            |
|                                                         | Talc (1)                  | 3.8 $\mu\text{m}$  | 3.3                                                                | Tabular form                        | 0.6                            |
| 112                                                     | Silica (7)                | 1.7 $\mu\text{m}$  | 1.0                                                                | Spherical form                      | 0.6                            |
| 113                                                     | Silica (7)                | 1.2 $\mu\text{m}$  | 20.9                                                               | Indeterminate form                  | 0.6                            |
| 114                                                     | Magnesium oxide (4)       | 1.2 $\mu\text{m}$  | 4.4                                                                | Tabular form                        | 5.6                            |
| 115                                                     | Magnesium oxide (4)       | 1.2 $\mu\text{m}$  | 4.4                                                                | Tabular form                        | 2.0                            |
| 116                                                     | Magnesium oxide (4)       | 1.2 $\mu\text{m}$  | 4.4                                                                | Tabular form                        | 0.015                          |
| 117                                                     | Magnesium oxide (4)       | 1.2 $\mu\text{m}$  | 4.4                                                                | Tabular form                        | 0.0008                         |

## (Preparation of Heat Sensitive Image-Receiving Sheet)

A paper support, on both sides of which polyethylene was laminated, was subjected to corona discharge treatment on the surface thereof, and then a gelatin undercoat layer containing sodium dodecylbenzenesulfonate was disposed on the treated surface. The subbing layer, the heat insulation layer, the lower receptor layer and the upper receptor layer each having the following composition were simultaneously multilayer-coated on the gelatin undercoat layer, in the state that the subbing layer, the heat insulation layer, the lower receptor layer and the upper receptor layer were laminated in this order from the side of the support, by a method illustrated in FIG. 9 in U.S. Pat. No. 2,761,791. The coating was performed so that coating amounts of the subbing layer, the heat insulation layer, the lower receptor layer, and the upper receptor layer after drying would be 6.0  $\text{g}/\text{m}^2$ , 8.5  $\text{g}/\text{m}^2$ , 2.4  $\text{g}/\text{m}^2$  and 3.0  $\text{g}/\text{m}^2$ , respectively.

## Upper receptor layer

|                                                                                                        |                 |
|--------------------------------------------------------------------------------------------------------|-----------------|
| Vinyl chloride-series latex<br>(trade name: Vinybran 900, manufactured by Nisshin Chemicals Co., Ltd.) | 21.0 mass parts |
| Vinyl chloride-series latex<br>(trade name: Vinybran 276, manufactured by Nisshin Chemicals Co., Ltd.) | 1.6 mass parts  |
| Gelatin (10% solution)                                                                                 | 2.5 mass parts  |
| The following ester-series wax EW-1                                                                    | 1.8 mass parts  |
| The following surfactant F-1                                                                           | 0.1 mass part   |
| The following surfactant F-2                                                                           | 0.4 mass part   |

|                                                                                                        |                 |
|--------------------------------------------------------------------------------------------------------|-----------------|
| Vinyl chloride-series latex<br>(trade name: Vinybran 690, manufactured by Nisshin Chemicals Co., Ltd.) | 18.0 mass parts |
| Vinyl chloride-series latex<br>(trade name: Vinybran 900, manufactured by Nisshin Chemicals Co., Ltd.) | 8.0 mass parts  |
| Gelatin (10% solution)                                                                                 | 8.0 mass parts  |
| The following surfactant F-1                                                                           | 0.03 mass part  |

25

-continued

| Heat insulation layer                                                                                                                                                                                                                                                                                                                               |                 |
|-----------------------------------------------------------------------------------------------------------------------------------------------------------------------------------------------------------------------------------------------------------------------------------------------------------------------------------------------------|-----------------|
| Hollow latex polymer particles<br>(trade name: MH5055, manufactured by Nippon Zeon Co., Ltd.)                                                                                                                                                                                                                                                       | 66.0 mass parts |
| Gelatin (10% solution)                                                                                                                                                                                                                                                                                                                              | 24.0 mass parts |
| Subbing layer                                                                                                                                                                                                                                                                                                                                       |                 |
| Polyvinyl alcohol<br>(trade name: POVAL PVA 205, manufactured by Kuraray)                                                                                                                                                                                                                                                                           | 7.0 mass parts  |
| Styrene butadiene rubber latex<br>(trade name: SN-307, manufactured by NIPPON A & L INC)                                                                                                                                                                                                                                                            | 55.0 mass parts |
| The following surfactant F-1                                                                                                                                                                                                                                                                                                                        | 0.02 mass part  |
| (EW-1)                                                                                                                                                                                                                                                                                                                                              |                 |
| $\begin{array}{c} \text{C}_{17}\text{H}_{35}-\text{OCO} \\   \\ \text{C}_{17}\text{H}_{35}\text{OCO} \end{array} \text{---} \text{O} \text{---} \begin{array}{c} \text{OCOC}_{17}\text{H}_{35} \\   \\ \text{OCOC}_{17}\text{H}_{35} \end{array}$                                                                                                   |                 |
| (F-1)                                                                                                                                                                                                                                                                                                                                               |                 |
| $\begin{array}{c} \text{O} \\    \\ \text{NaO}_3\text{S} \text{---} \text{CH}_2 \text{---} \text{C}(\text{O}) \text{---} \text{O}(\text{CH}_2)_2(\text{CF}_2)_3\text{CF}_3 \\ \text{O} \\    \\ \text{NaO}_3\text{S} \text{---} \text{CH}_2 \text{---} \text{C}(\text{O}) \text{---} \text{O}(\text{CH}_2)_2(\text{CF}_2)_3\text{CF}_3 \end{array}$ |                 |
| F-2                                                                                                                                                                                                                                                                                                                                                 |                 |
| $\begin{array}{c} \text{C}_2\text{H}_5 \\   \\ \text{CH}_2\text{CO}_2\text{CHCH}_2\text{C}_4\text{H}_9 \\   \\ \text{NaO}_3\text{S} \text{---} \text{CHCH}_2\text{O}_2\text{CH}_2\text{CHC}_4\text{H}_9 \\   \\ \text{C}_2\text{H}_5 \end{array}$                                                                                                   |                 |

## (Formation, Measurement and Evaluation of Images)

The heat-sensitive transfer sheet (101) and the heat-sensitive transfer image-receiving sheet, 152 mm  $\times$  102 mm in size, were used to output a black solid image on the image-receiving sheet by means of a heat transfer type printer. It was

understood that low-temperature and low-humidity conditions causes a large deformation of such heat-sensitive transfer sheets and give a large amount of dirt or stains adhering to the thermal printer head of a printer; therefore, environmental conditions for outputting the image were set to low-temperature and low-humidity conditions of 15° C. in temperature and 20% in relative humidity (R.H.).

The image-printing resolution of the heat transfer type printer was 300 dpi. The yellow, magenta, and cyan recording energies were each set to 2.5 J/cm<sup>2</sup>, and the line speed was set to 1.5 msec/line and 0.6 msec/line. The highest arrival temperature of the thermal printer head (TPH) was 420° C. The length of the heat-sensitive transfer sheet was measured before and after the image was printed. The length of the elongation of the sheet was calculated by subtracting the sheet length before the printing from the sheet length after the printing. Furthermore, the elongation ratio was calculated by dividing the length of the elongation by the length of the image-printed area. As this value is smaller, the heat-sensitive transfer sheet is less deformed so that defects are less generated in the outputted image.

Under the same conditions as described above, images were continuously outputted on 300 sheets. Thereafter, a

color 3D laser microscope (trade name: VK-9500 GII, manufactured by Keyence Corp.) was used to analyze the profile of the shape of the thermal printer head, and measure the height of the profile. In this way, the height of the adhering dirt and stains was obtained. As this value is smaller, the amount of the material adhering to the thermal printer head is smaller so that the heat-sensitive transfer sheet is further restrained from being cut. Simultaneously, the thermal printer head surface was observed with a microscope to judge the state of injures or shaven regions therein on the following criterion.

(Criterion)

- 1: No injures or shaven regions are generated.
- 2: Injures or shaven regions are slightly generated but are allowable.
- 3: Deep injures are present in places, and shaven regions are slightly present.
- 4: Deep injures and deep shaven regions are present.

As the criterion number is smaller, the state of the thermal printer head is better.

The evaluation results are shown in Table 23 described below.

TABLE 23

| Heat-sensitive transfer sheet sample name | Elongation of the heat-sensitive transfer sheet (%) |             | State of thermal printer head |             |                                          |             | Remarks             |  |
|-------------------------------------------|-----------------------------------------------------|-------------|-------------------------------|-------------|------------------------------------------|-------------|---------------------|--|
|                                           |                                                     |             | Stain height (μm)             |             | Evaluation of injures and shaven regions |             |                     |  |
|                                           | 1.5 ms/line                                         | 0.6 ms/line | 1.5 ms/line                   | 0.6 ms/line | 1.5 ms/line                              | 0.6 ms/line |                     |  |
| 101                                       | 2.5                                                 | 5.5         | 0.8                           | 3.5         | 1                                        | 1           | Comparative example |  |
| 102                                       | 1.2                                                 | 5.4         | 0.7                           | 3.3         | 1                                        | 1           | Comparative example |  |
| 103                                       | 1.2                                                 | 3.7         | 0.7                           | 3.6         | 1                                        | 3           | Comparative example |  |
| 104                                       | 1.3                                                 | 2.0         | 0.6                           | 1.9         | 1                                        | 1           | This invention      |  |
| 105                                       | 1.1                                                 | 1.7         | 0.7                           | 1.3         | 1                                        | 1           | This invention      |  |
| 106                                       | 1.9                                                 | 6.0         | 0.7                           | 2.8         | 3                                        | 4           | Comparative example |  |
| 107                                       | 1.3                                                 | 1.8         | 0.6                           | 1.4         | 1                                        | 2           | This invention      |  |
| 108                                       | 1.2                                                 | 1.9         | 0.7                           | 1.7         | 1                                        | 1           | This invention      |  |
| 109                                       | 2.7                                                 | 5.6         | 0.7                           | 3.4         | 1                                        | 1           | Comparative example |  |
| 110                                       | 1.9                                                 | 2.0         | 0.8                           | 1.9         | 1                                        | 2           | This invention      |  |
| 111                                       | 1.0                                                 | 1.1         | 0.7                           | 0.9         | 1                                        | 1           | This invention      |  |
| 112                                       | 1.8                                                 | 6.8         | 0.8                           | 3.3         | 1                                        | 1           | Comparative example |  |
| 113                                       | 1.4                                                 | 1.9         | 0.8                           | 1.8         | 2                                        | 2           | This invention      |  |
| 114                                       | 1.7                                                 | 1.9         | 0.8                           | 1.3         | 3                                        | 3           | Comparative example |  |
| 115                                       | 1.2                                                 | 1.4         | 0.7                           | 1.4         | 1                                        | 1           | This invention      |  |
| 116                                       | 1.7                                                 | 2.1         | 0.8                           | 1.9         | 1                                        | 1           | This invention      |  |
| 117                                       | 2.3                                                 | 5.4         | 0.8                           | 3.5         | 1                                        | 1           | Comparative example |  |

The following are understood from Table 23: in the sample (102), wherein inorganic particles having a Mohs' hardness outside the range in the invention were used, the elongation of the heat-sensitive transfer sheet was restrained in low-speed printing but the elongation was not restrained in high-speed print as compared with situations in the sample (101). In the samples (103) and (112), wherein the ratio of the particle maximum width to the sphere equivalent diameter was outside the range in the invention, and the samples (106) and (109), wherein the mean particle size was outside the range in the invention, the effect of restraining the elongation of the heat-sensitive transfer sheets was insufficient or rather deteriorated in high-speed print. Furthermore, the thermal printer head was more largely injured in some of these samples. In the sample (114), wherein the amount of used inorganic particles was larger than the range in the invention, injures in the thermal printer head deteriorated. In the sample (117), wherein the amount of used inorganic particles was smaller than the range in the invention, the effect of restraining the elongation of the heat-sensitive transfer sheet was not pro-

duced and the effect of decreasing stains on the thermal printer head was not produced, either. In the samples (104), (105), (107), (108), (110), (111), (113), (115) and (116), wherein inorganic particles satisfying the ranges specified in the invention were used, the elongation of the heat-sensitive transfer sheets was restrained even in high-speed print, and further stains, injures and shaven regions were less generated in the thermal printer head.

Having described our invention as related to the present embodiments, it is our intention that the invention not be limited by any of the details of the description, unless otherwise specified, but rather be construed broadly within its spirit and scope as set out in the accompanying claims.

This non-provisional application claims priority under 35 U.S.C. §119 (a) on Patent Application No. 2007-255793 filed in Japan on Sep. 28, 2007, which is entirely herein incorporated by reference.

What I claim is:

1. A heat-sensitive transfer sheet comprising a base film, a dye layer formed over one surface of the base film and con-

55

taining a heat-transferable dye and a resin, and a heat-resistant lubricating layer formed over the other surface of the base film and containing inorganic particles and a resin, wherein the inorganic particles contained in the heat-resistant lubricating layer have a Mohs' hardness of 3 to 7 and a mean particle size of 0.3 to 5  $\mu\text{m}$ , the ratio of the maximum width of each of the inorganic particles to the sphere equivalent diameter thereof is from 1.5 to 50, and the ratio of the contained inorganic particles to the total coating amount of the heat-resistant lubricating layer is from 0.001 to 5 mass %.

2. The heat-sensitive transfer sheet according to claim 1, wherein the Mohs' hardness ranges from 3 to 6.

3. The heat-sensitive transfer sheet according to claim 1, wherein the shape of the inorganic particles is tabular.

4. The heat-sensitive transfer sheet according to claim 1, wherein the inorganic particles contain particles in at least two forms which include tabular particles and needle particles.

5. The heat-sensitive transfer sheet according to claim 1, wherein the ratio of the mass of the inorganic particles to the total coating mass of the heat-resistant lubricating layer is from 0.01% to 2 mass %.

6. The heat-sensitive transfer sheet according to claim 1, wherein the inorganic particles are made of magnesium oxide.

7. The heat-sensitive transfer sheet according to claim 1, wherein the above-described heat-sensitive transfer sheet contains at least one dye represented by any one of following formulae (Y1) to (Y9) set forth below:



Formula (Y1)

wherein the ring A represents a substituted or unsubstituted benzene ring; R<sup>1</sup> and R<sup>2</sup> each independently represent a hydrogen atom, a substituted or unsubstituted alkyl group, a substituted or unsubstituted alkenyl group or a substituted or unsubstituted aryl group; R<sup>3</sup> represents a hydrogen atom, a substituted or unsubstituted alkyl group, a substituted or unsubstituted amino group, a substituted or unsubstituted alkoxy group, a substituted or unsubstituted aryloxycarbonyl group, a substituted or unsubstituted aryloxycarbonyl group, a substituted or unsubstituted aryl group, or a substituted or unsubstituted carbamoyl group; and R<sup>4</sup> represents a substituted or unsubstituted alkyl group, or a substituted or unsubstituted aryl group;



Formula (Y2)

56

wherein R<sup>5</sup> represents a substituted or unsubstituted alkyl group, or a substituted or unsubstituted alkenyl group, R<sup>6</sup> and R<sup>7</sup> each independently represent a substituted or unsubstituted alkyl group, R<sup>8</sup> represents a substituted or unsubstituted alkyl group, a substituted or unsubstituted aryl group, a substituted or unsubstituted alkoxy group, or a substituted or unsubstituted amino group, and R<sup>9</sup> represents a substituted or unsubstituted alkyl group, or a substituted or unsubstituted aryl group;



Formula (Y3)

wherein R<sup>10</sup> represents a hydrogen atom, or a substituted or unsubstituted alkyl group, R<sup>11</sup> represents a hydrogen atom or a halogen atom, and R<sup>12</sup> represents a substituted or unsubstituted aryloxycarbonyl group, a substituted or unsubstituted aryloxycarbonyl group, or a substituted or unsubstituted carbamoyl group;



Formula (Y4)

wherein the ring B represents a substituted or unsubstituted aryl group, or a substituted or unsubstituted aromatic heterocyclic group, R<sup>13</sup> represents a substituted or unsubstituted alkyl group, and R<sup>14</sup> represents a substituted or unsubstituted alkyl group, or a substituted or unsubstituted aryl group;



Formula (Y5)

wherein R<sup>15</sup>, R<sup>16</sup>, R<sup>17</sup> and R<sup>18</sup> each independently represent a substituted or unsubstituted alkyl group or a substituted or unsubstituted aryl group;



Formula (Y6)

57

wherein the rings C, D and E each independently represent a substituted or unsubstituted benzene ring;



Formula (Y7) 5

wherein the ring F represents a substituted or unsubstituted benzene ring; and R¹⁹ and R²⁰ each independently represent a hydrogen atom, a substituted or unsubstituted alkyl group, a substituted or unsubstituted alkenyl group or a substituted or unsubstituted aryl group;



Formula (Y8)

wherein the ring G represents a substituted or unsubstituted benzene ring; and R²¹ and R²² each independently represent a hydrogen atom or a substituted or unsubstituted alkyl group; and



Formula (Y9)

wherein R²³ represents a substituted or unsubstituted alkyl group or a substituted or unsubstituted alkenyl group.

8. The heat-sensitive transfer sheet according to claim 1, wherein the above-described heat-sensitive transfer sheet contains at least one dye represented by any one of following formulae (M1) to (M8) set forth below:



Formula (M1) 50

wherein the ring H represents a substituted or unsubstituted benzene ring or a substituted or unsubstituted pyridine ring; and R²⁴, R²⁵, R²⁶ and R²⁷ each independently represent a substituted or unsubstituted alkyl group, a substituted or unsubstituted alkenyl group or a substituted or unsubstituted aryl group;



Formula (M2)

wherein the ring I represents a substituted or unsubstituted benzene ring or a substituted or unsubstituted pyridine ring; and R²⁸, R²⁹, R³⁰ and R³¹ each independently represent a substituted or unsubstituted alkyl group, a substituted or unsubstituted alkenyl group or a substituted or unsubstituted aryl group;



Formula (M3)

wherein the ring J represents a substituted or unsubstituted benzene ring, and R³², R³³ and R³⁴ each independently represent a substituted or unsubstituted alkyl group, a substituted or unsubstituted alkenyl group or a substituted or unsubstituted aryl group;



Formula (M4)

wherein the ring K represents a substituted or unsubstituted benzene ring, and R³⁵, R³⁶ and R³⁷ each independently represent a substituted or unsubstituted alkyl group, a substituted or unsubstituted alkenyl group or a substituted or unsubstituted aryl group;



Formula (M5)

wherein R³⁸ and R³⁹ each independently represent a substituted or unsubstituted alkyl group, a substituted or unsubstituted aryl group, or a substituted or unsubstituted heterocyclic group, and R⁴⁰ and R⁴¹ each independently represent a substituted or unsubstituted alkyl group, a substituted or unsubstituted alkenyl group, or a substituted or unsubstituted aryl group;

59



Formula (M6)

60

halogen atom, R<sup>48</sup> represents a substituted or unsubstituted alkyl group, R<sup>49</sup> represents a substituted or unsubstituted acylamino group or a substituted or unsubstituted alkoxy carbonylamino group, and R<sup>50</sup> and R<sup>51</sup> each independently represent a substituted or unsubstituted alkyl group, a substituted or unsubstituted alkenyl group or a substituted or unsubstituted aryl group;



Formula (C2)

wherein R<sup>42</sup> is a substituted or unsubstituted aryloxy group, R<sup>43</sup> is a hydrogen atom, or a substituted or unsubstituted aryloxy group, and R<sup>44</sup> is a hydroxyl group, or a substituted or unsubstituted amino group;



Formula (M7)

wherein the ring L represents a substituted or unsubstituted benzene ring; and R<sup>45</sup> and R<sup>46</sup> each independently represent a hydrogen atom, a substituted or unsubstituted alkyl group, a substituted or unsubstituted alkenyl group or a substituted or unsubstituted aryl group; and



Formula (M8)

wherein the ring Q represents a substituted or unsubstituted benzene ring, R<sup>100</sup> represents a substituted or unsubstituted alkyl group, a substituted or unsubstituted aryl group, a substituted or unsubstituted alkoxy group, or a substituted or unsubstituted amino group, R<sup>101</sup> represents a substituted or unsubstituted alkyl group, or a substituted or unsubstituted aryl group, R<sup>102</sup> and R<sup>103</sup> each independently represent a hydrogen atom, a substituted or unsubstituted alkyl group, a substituted or unsubstituted alkenyl group, or a substituted or unsubstituted aryl group.

9. The heat-sensitive transfer sheet according to claim 1, wherein the above-described heat-sensitive transfer sheet contains at least one dye represented by any one of following formulae (C1) to (C4) set forth below:



Formula (C1)

wherein the ring M represents a substituted or unsubstituted benzene ring, R<sup>47</sup> represents a hydrogen atom or a

wherein the ring N represents a substituted or unsubstituted benzene ring, R<sup>52</sup> represents a hydrogen atom, a substituted or unsubstituted acylamino group, a substituted or unsubstituted alkoxy carbonyl group, or a substituted or unsubstituted carbamoyl group, and R<sup>53</sup> and R<sup>54</sup> each independently represent a substituted or unsubstituted alkyl group, a substituted or unsubstituted alkenyl group, or a substituted or unsubstituted aryl group;



Formula (C3)

wherein R<sup>55</sup> and R<sup>56</sup> each independently represent an alkyl group, or a substituted or unsubstituted aryl group; and



Formula (C4)

wherein the ring O represents a substituted or unsubstituted benzene ring, and R<sup>57</sup> and R<sup>58</sup> each independently represent a substituted or unsubstituted alkyl group, a substituted or unsubstituted alkenyl group, or a substituted or unsubstituted aryl group.

10. An image formation method in which images are formed in a state that the heat-sensitive transfer sheet according to claim 1 is superposed upon a heat-sensitive transfer image-receiving sheet having at least one dye-receiving layer on a support.

11. The image formation method according to claim 10, wherein the heat-sensitive transfer image-receiving sheet has at least one dye-receiving layer on a support, and further has at least one heat insulation layer containing hollow polymeric particles and a hydrophilic polymer between the dye-receiving layer and the support.

\* \* \* \* \*